# EUROPEAN PATENT SPECIFICATION

(11) **EP 2 487 042 B1**
(45) Date of publication and mention of the grant of the patent: **03.09.2014**
(21) Application number: 09847000.8
(22) Date of filing: 22.10.2009
(51) Int. Cl.: B41M 5/40, B44C 1/16, B44C 1/17, B44C 3/02, B41M 7/00

(54) **ULTRAVIOLET CURING TRANSFER FILM, MANUFACTURING METHOD THEREFOR AND APPLICATION THEREOF**
UV-HÄRTENDE TRANSFERFOLIE, VERFAHREN ZU IHRER HERSTELLUNG UND ANWENDUNG
FILM DE TRANSFERT À DURCISSEMENT AUX ULTRAVIOLETS, PROCÉDÉ DE FABRICATION ET APPLICATION DE CELUI-CI

(30) Priority: 06.07.2009 CN 200910088641
(43) Date of publication of application: 15.08.2012
(73) Proprietor: Zhuhai Dongcheng UV Materials Co., Ltd., Guangdong 519050 (CN)
(72) Inventor: CHEN, Wei, Zhuhai Guangdong 519050 (CN); TAN, Haoya, Zhuhai Guangdong 519050 (CN); ZHOU, Lihui, Zhuhai Guangdong 519050 (CN)
(74) Representative: Intès, Didier Gérard André
(86) International application number: PCT/CN2009/074567
(87) International publication number: WO 2011/003249

(56) References cited:
- WO-A2-2009/013580
- CN-A- 101 235 672
- CN-A- 101 348 047
- CN-Y- 2 573 236
- CN-Y- 200 995 575
- CN-Y- 201 176 036
- CN-Y- 201 209 305
- GB-A- 2 010 184
- JP-A- 9 078 473
- JP-A- H0 978 473
- JP-A- 10 157 399
- US-A- 1 895 419
- US-A- 5 560 796
- US-A- 6 022 050
- US-A1- 2007 129 249
- US-A1- 2007 142 492
- US-A1- 2009 046 134
- US-B1- 6 284 327

## Description

### Field of the Invention

The present invention pertains to the finishing material field, in particular relates to an UV-curing transfer film or colorful transfer film produced by uniformly spreading or printing UV-curable paint/ink (abbreviated as UV paint/ink), and a preparation method and an application of the UV-curing transfer film or colorful transfer film.

### Background of the Invention

Nowadays, as interior and exterior finishing products become luxury increasingly and the requirements of the state for environmental protection, energy conservation, and sustainable development become higher and higher, the criteria for energy conservation and emission reduction in production and construction procedures become more and more stringent. At present, existing transfer films for interior and exterior finishing products are usually thermal transfer films or aqueous transfer films. However, thermal transfer films or aqueous transfer films involve volatilization of a great deal of organic solvent and heavy exhaust pollution, as described in CN101318420; moreover, when thermal transfer films or aqueous transfer films are applied to timber boards, cement boards, gypsum boards, or metal plates, thermal transfer films or aqueous transfer films tend to peel off from the boards or plates. Photo-cured paint is a sort of green paint free of volatile organic compounds, and UV-curable paint or UV-curable ink has advantages such as high curing rate, low energy consumption, low equipment investment, small equipment footprint, and high film performance, etc.; therefore, the application of UV-curable colorful transfer films can bring more benefits.

For example, Patent Document US 5560796 A discloses a UV curing transfer sheet suitably for the decoration of ceramics, glassware or other objects.

Said UV-curing transfer sheet comprises a substrate film, a release agent layer, a UV-curing ink decorative pattern layer and a UV-curing ink background layer. The substrate film can be made of polypropylene, polyethylene, polyvinyl chloride or polyethylene terephthalate. The chemical composition of the ink used corresponds to the composition of the ink indicated in claim 1.

Similarly, Patent Document JP H09 784731 discloses a UV-curing transfer film for the decoration of cloth.

### Summary of the Invention

An object of the present invention is to provide an UV-curing transfer film or UV-curable colorful transfer film, which is rich in colors and patterns, and has high decorative and protective performance.

Another object of the present invention is to provide a method for preparation of UV-curing transfer film or UV-curable colorful transfer film.

Another object of the present invention is to provide an application of UV-curing transfer film or UV-curable colorful transfer film.

"A UV-curing transfer film according to the present invention is defined according to claim 1 in the appended set of claims."

The release agent layer can be coated or printed to required thickness, preferably 1~100µm thickness.

The UV-curable paint protective layer can be coated or printed to required thickness, preferably 1~100µm thickness.

The UV-curable ink decorative pattern layer can be coated or printed to required thickness, preferably 1~100µm thickness.

The UV-curable paint background layer can be coated or printed to required thickness, preferably 1~100µm thickness.

Calculated in weight percentage, the release agent that is used to produce the release agent layer is a mixture of 20~50% cellulose, 1~30% wax, 0~10% silicone oil, 0~10% (preferably 10~20%), 0~15% ethyl acetate (preferably 5~15%), 5~20% acrylate prepolymer, 5~20% acrylate monomer, and 1~6% photoinitiator.

Calculated in weight percentage, the UV-curable paint that is used to produce the UV-curable paint protective layer is:
A. mixture of 10~80% acrylate prepolymer, 5~50% acrylate monomer, 1~6% photoinitiator, 0~2% auxiliary agent, 0~50% filler, 0~10% butanone, and 0~15% ethyl acetate; or
B. mixture of 10~80% acrylate prepolymer, 5~50% acrylate monomer, 1~6% photoinitiator, 0~2% auxiliary agent, 0~50% filler, 1~50% matting agent, 0~10% butanone, and 0~15% ethyl acetate.

Calculated in weight percentage, the UV-curable ink that is used to produce the UV-curable ink decorative pattern layer is a mixture of 10~60% acrylate prepolymer, 5~50% acrylate monomer, 1~5% photoinitiator, 0~2% auxiliary agent, 0~50% filler, 5~30% toner, 5~30% resin, 0~10% butanone, and 0~15% ethyl acetate.

Calculated in weight percentage, the UV-curable paint that is used to produce the UV-curable paint background layer is a mixture of 10~50% acrylate prepolymer, 10~40% acrylate monomer, 1~5% photoinitiator, 0~2% auxiliary agent, 0~30% filler, 5~30% toner, 5~50% resin, 0~10% butanone, and 0~15% ethyl acetate.

The substrate film is any of polypropylene film, polyethylene film, polyvinyl chloride film, and polyethylene terephthalate film.

The polypropylene film can be a modified polypropylene film.

The cellulose can be methylol cellulose.

The wax can be modified paraffin wax, palm wax, or a mixture of them.

The silicone oil can be selected from at least one compound in the group of methyl-silicone oil, phenyl methyl silicone oil, and hydroxyl silicone oil, etc.

The acrylate prepolymer can be selected from at least one compound in the group of epoxy acrylate, fluorine-containing epoxy acrylate, polyurethane acrylate, fluorine-containing polyurethane acrylate, polyester acrylate, fluorine-containing polyester acrylate, amino acrylate, fluorine-containing amino acrylate, acrylate copolymer, and fluorine-containing acrylate copolymer, etc.

The acrylate monomer can be: (1) mono-functional monomer, such as butyl acrylate, cyclohexyl acrylate, ethylhexyl acrylate (EHA), hydroxyethyl acrylate (HEA), hydroxyethyl methacrylate (HEMA), trifluoro ethyl acrylate, trifluoro ethyl methacrylate, hexafluoro butyl acrylate, hexafluoro butyl methacrylate, dodecafluoro heptyl acrylate, or dodecafluoro heptyl methacrylate, etc.; (2) bi-functional monomer, such as tripropylene glycol diacrylate (TPGDA), dipropylene glycol diacrylate (DPGDA), neopentyl glycol diacrylate (NPGDA), propoxy-neopentyl glycol diacrylate (PO-NPGDA), phthalandione di-(diethylene glycol) diacrylate (PDDA), or 1, 6-ethylene glycol diacrylate (HDDA), etc.; (3) poly-functional monomer, such as trimethylolpropane triacrylate (TMPTA), ethoxy- trimethylolpropane triacrylate (EO-TMPTA), propoxy-trimethylolpropane triacrylate (PO-TMPTA), pentaerythritol triacrylate (PETA), or dipentaerythritol hexa-acrylate (DPHA), etc., and is usually selected from at least one compound in any above group of acrylate monomers.

The resin can be selected from at least one compound in the group of modified polyvinyl acetate, polyamide resin, thermoplastic acrylic, etc.

The modified polyvinyl acetate can be vinyl chloride vinyl acetate, ethylene vinyl acetate, or a mixture of them.

The photoinitiator can be selected from at least one compound in the group of benzoin ether photoinitiator, benzil ketal photoinitiator, acetophenone photoinitiator, anthraquinone photoinitiator, thioxanthone photoinitiator, benzophenone photoinitiator, acyl phosphine oxide photoinitiator, and benzoate photoinitiator.

The benzoin ether photoinitiator can be selected from at least on compound in the group of benzoin methyl ether, benzoin ethyl ether, and benzoin isopropyl ether, etc.

The benzil ketal photoinitiator can be benzil dimethyl ketal, etc.

The acetophenone photoinitiator can be selected from at least one compound in the group of acetophenone, 2, 2-dimethoxy-2-phenyl acetophenone, 2, 2-diethoxy-2-phenyl acetophenone, 1, 1-dichloroacetophenone, 1-hydroxyl acetophenone, 1-hydroxyl cyclohexyl phenyl ketone, 2-hydroxyl-2-methyl-1-phenyl-1-acetone, 1-(4-isopropyl phenyl)-2-hydroxyl-2-methyl-1-acetone, 1-[4-(2-hydroxyl ethyoxyl) phenyl]-2-hydroxyl-2-methyl-1-acetone, 2-methyl-1-[4-(methyl sulfenyl) phenyl]-2-morpholinyl-1-acetone, and 2-benzyl-2-dimethyl amido-1-(4-morpholinyl phenyl)-1-butanone.

The anthraquinone photoinitiator can be selected from at least one compound in the group of 2-tertiary butyl anthraquinone, 1-chlorine anthraquinone, and 2-amyl anthraquinone.

The thioxanthone photoinitiator can be selected from at least one compound in the group of 2, 4-dimethyl thioxanthone, 2, 4-diethyl thioxanthone, 2-isopropyl thioxanthone, 4-isopropyl thioxanthone, 2-chloro-thioxanthone, and 2, 4-diisopropyl thioxanthone, etc.

The benzophenone photoinitiator can be selected from at least one compound in the group of diphenyl ketone, 4-chlorine diphenyl ketone, methyl benzophenone, and 4-benzoyl-4'-methyl diphenyl thioether, etc.

The acyl phosphine oxide photoinitiator can be selected from at least one compound in the group of 2, 4, 6-trimethyl benzoyl diphenyl phosphine oxide, di-(2, 4, 6-trimethyl benzoyl)-phenyl phosphine oxide, di-(2, 6-dimethyl benzoyl)-2, 4, 4-trimethyl amyl phosphine oxide, 2, 4, 6-trimethyl benzoyl phenyl ethyoxyl phosphine oxide, etc.

The benzoate photoinitiator can be methyl benzoyl benzoate, methyl ortho-benzoyl. benzoate, or a mixture of them.

The auxiliary agent is preferably selected from at least one compound in the group of flatting agent from BKY Additives & Instruments (e.g., BYK306, BYK358, or a mixture of them), anti-foaming agent from BKY Additives & Instruments (e.g., BYK052, BYK055, or a mixture of them), and wetting and dispersing agent from BKY Additives & Instruments (e..g, Disperbyk 103, Disperbyk 163, or a mixture of them). The filler can be selected from at least one compound in the group of talcum powder, calcium carbonate, and barium sulfate, etc.

The toner can be selected from at least one in the group of soot carbon, titanium pigment, titanium cyanine, proflavine, and scarlet powder, etc.

The matting agent is matting wax (preferably the matting wax from Japan GIFU), matting powder, or a mixture of them.

"A method for producing a UV-curing transfer film according to the present invention is defined according to claim 7 in the appended set of claims."

The substrate film used in the present invention can be pre-treated, by baking at a temperature within 60~200°C range determined according to the material of the substrate film, to force the substrate film to pre-shrink, and remove electrostatic charges.

The curing process under infrared irradiation is: adjust the infrared heating temperature to 20~150°C, let the release agent to flow flat for 0.01~10min., and cure the release agent completely.

The curing process under UV irradiation is: expose the paint/ink to UV irradiation from 1-3 ultraviolet lamps (high-voltage mercury lamps) with 2-20Kw unit power and 0~3 metal halide lamps (iodine gallium lamps, iron lamps, or dysprosium lamps, etc.) with 3~20Kw unit power in an UV curing machine, at 200-600nm wavelength, to cure the UV-curable protective paint, UV-curable ink, and UV-curable background color paint, with the UV curing machine operating at 1~200m/min. conveying speed.

The UV-curing transfer film or UV-curable colorful transfer film provided in the present invention is available in a variety of colors, patterns, and textures, including: colorful transfer film with masonry texture (e.g., artificial marble or granite), colorful transfer film with timber texture, colorful transfer film with brushed metal effect, colorful transfer film with mirror metal effect, colorful transfer film with crystal effect, colorful transfer film with character or cartoon images, colorful transfer film with poetry images, colorful transfer film with plant and animal images, and colorful transfer film with landscape images, etc. The UV-curing transfer film or UV-curable colorful transfer film provided in the present invention can be used as a decorative material for various indoor or outdoor products.

UV-curing transfer films or UV-curable colorful transfer films obtained with the preparation method provided in the present invention have advantages such as high material strength, high weather resistance, environmental protection, rich colors and patterns, full and rigid paint film, high scratch resistance, easy cleaning, and non-flammability, etc., and have better decorative and protective performance than existing thermal transfer films and aqueous transfer films.

The UV-curing transfer film or UV-curable colorful transfer film provided in the present invention can be used to produce UV curing transfer film decorative boards.

The application described in the present invention is: apply a layer of UV-curable permeating agent (e.g., the UV-curable permeating agent disclosed in Patent Application No. CN200710120791.1) on the surface of a substrate, such as fiber reinforced cement board, fiber reinforced calcium silicate board, fiber reinforced magnesium oxide board, light-weight magnesium chloride cement board, magnesium oxychloride board, or gypsum board, apply a layer of UV-curable paint filler on the surface of the UV-curable permeating agent, apply a layer of UV-curable sealing prime varnish on the surface of the UV-curable paint filler, apply a layer of UV-curable pigmented paint on the surface of the UV-curable sealing prime varnish, apply a layer of UV-curable glue on the surface of the UV-curable pigmented paint, and transfer a transfer film onto the UV-curable glue (the transfer film can be transferred with a transfer machine onto the surface of a decorative board that is coated with UV-curable glue), to obtain an UV-curing transfer film decorative board; or

Apply a layer of UV-curable sealing clear prime paint on the surface of a substrate (e.g., solid timber board, medium density fiberboard, or plywood board), apply a layer of UV-curable glue on the surface of the UV-curable sealing clear prime paint, and transfer a transfer film onto the surface of the UV-curable glue (the transfer film can be transferred with a transfer machine to the surface of a decorative board that is coated with UV-curable glue), to obtain an UV-curing transfer film decorative board; or Apply a layer of UV-curable metal prime paint on the surface of a substrate (e.g., aluminum plate, steel plate, or iron plate), apply a layer of UV-curable glue on the surface of the UV-curable metal prime paint, and transfer a transfer film onto the surface of the UV-curable glue (the transfer film can be transferred with a transfer machine to the surface of a decorative plate that is coated with UV-curable glue), to obtain an UV-curing transfer film decorative plate.

The UV-curable permeating agent can be coated by roller coating or brush painting, at a rate of 50~50g/m², to provide high anchoring, waterproof, and alkali-resistant effect; after cured, the UV-curable permeating agent is incorporated into the substrate, so as to increase the strength of the substrate, ensure firm bonding between the paint film and the substrate, and thereby ensure the service life of the decorative board/plate.

The UV-curable paint filler can be coated by roller coating or blade coating, to 10~150µm thickness.

The UV-curable sealing clear prime paint can be coated by roller coating, flow coating, or spray coating, to 10~150µm thickness.

The UV-curable pigmented paint can be coated by roller coating, flow coating, or spray coating, to 10~150µm thickness.

The UV-curable metal prime paint can be coated by roller coating, flow coating, or spray coating, to 2~150µm thickness.

The UV-curable glue can be coated by roller coating or spray coating, to 2~150µm thickness.

The UV-curing transfer film decorative board/plate in the present invention can be obtained with the following preparation method:
(1) Surface treatment of the substrate;
(2) Coat UV-curable permeating agent on the substrate prepared in step (1);
(3) Let the coating to flow flat under infrared irradiation or naturally;
(4) Coat UV-curable paint filler on the substrate prepared in step (3);
(5) Cure under UV irradiation;
(6) Coat UV-curable sealing clear prime paint on the substrate prepared in step (5);
(7) Cure under UV irradiation;
(8) Sanding and dust removing;
(9) Coat UV-curable sealing clear prime paint on the substrate prepared in step (8);
(10) Cure under UV irradiation;
(11) Coat UV-curable pigmented paint on the substrate prepared in step (10);
(12) Let the coating to flow flat under infrared irradiation or naturally;
(13) Cure under UV irradiation;
(14) Sanding and dust removing;
(15) Coat UV-curable glue on the substrate prepared in step (14);
(16) Cure under UV irradiation;
(17) Transfer a transfer film onto the substrate prepared in step (16);
(18) Cure under UV irradiation;
(19) Remove the film;
(20) Let the coating to flow flat under infrared irradiation;
(21) Coat UV-curable glue on the substrate prepared in step (20);
(22) Cure under UV irradiation;
(23) Coat UV-curable protective varnish on the substrate prepared in step (22);
(24) Let the coating to flow flat under infrared irradiation or naturally;
(25) Cure under UV irradiation;
(26) Inspection;
(27) Apply a protective film;
(28) Packaging

The steps 19~27 can be omitted, since the transfer film itself has a protective layer. Or
(1) Surface treatment of the substrate;
(2) Coat UV-curable sealing clear prime paint on the substrate prepared in step (1);
(3) Cure under UV irradiation;
(4) Sanding and dust removing;
(5) Coat UV-curable glue on the substrate prepared in step (4);
(6) Cure under UV irradiation;
(7) Transfer a transfer film onto the substrate prepared in step (6);
(8) Cure under UV irradiation;
(9) Remove the film;
(10) Let the coating to flow flat under infrared irradiation;
(11) Coat UV-curable glue on the substrate prepared in step (10);
(12) Cure under UV irradiation;
(13) Coat UV-curable protective varnish on the substrate prepared in step (12);
(14) Let the coating to flow flat under infrared irradiation or naturally;
(15) Cure under UV irradiation;
(16) Inspection;
(17) Apply a protective film;
(18) Packaging

The steps 9-17 can be omitted, since the transfer film itself has a protective layer. Or
(1) Surface treatment of the substrate;
(2) Coat UV-curable metal prime paint on the substrate prepared in step (1);
(3) Cure under UV irradiation;
(4) Coat UV-curable glue on the substrate prepared in step (3);
(5) Cure under UV irradiation;
(6) Transfer a transfer film onto the substrate prepared in step (5);
(7) Cure under UV irradiation;
(8) Remove the film;
(9) Let the coating to flow flat under infrared irradiation;
(10) Coat UV-curable glue on the substrate prepared in step (9);
(11) Cure under UV irradiation;
(12) Coat UV-curable protective varnish on the substrate prepared in step (11);
(13) Let the coating to flow flat under infrared irradiation or naturally;
(14) Cure under UV irradiation;
(15) Inspection;
(16) Apply a protective film;
(17) Packaging

The steps 8~16 can be omitted, since the transfer film itself has a protective layer. Surface treatment of the substrate: treat the substrate by sanding, and remove dust from the surface of the substrate.

Coat UV-curable permeating agent: coat UV-curable permeating agent by roller coating or brush painting, at a coating rate of 50~500g/m².

Let the coating to flow flat under infrared irradiation or naturally: adjust the temperature in the infrared flatting machine to 20~150°C, and let the coating to flow flat for 0.1~10min., and let the solvent in the coat to volatilize fully; if natural flatting is used, hold the coated work piece for 1min.~24h under natural conditions, to let the coating to flow flat and the solvent in the coating to volatilize fully.

Coat UV-curable paint filler: coat UV-curable paint filler by roller coating or blade coating, to 10~150µm thickness.

Cure under UV irradiation: load the coated work piece into an UV curing machine equipped with 1~3 ultraviolet tubes (high-voltage mercury lamps) with 3~20Kw unit power and 0-3 metal halide lamps (iodine gallium lamps, iron lamps, or dysprosium lamps, etc.) with 3~20Kw unit power, and cure the coating under UV irradiation, at 200~600nm wavelength, with the UV curing machine operating at 5~50m/min. conveying speed.

Coat UV-curable sealing clear prime paint: coat UV-curable sealing clear prime paint by roller coating, flow coating, or spray coating, to 10~150µm thickness.

Sanding and dust removing: treat the work piece in a sanding machine, with an 80~800-mesh abrasive belt, and remove the dust from the surface of the work piece. Coat UV-curable sealing clear prime paint: coat UV-curable sealing clear prime paint by roller coating, flow coating, or spray coating, to 5~50µm thickness.

Coat UV-curable pigmented paint: coat UV-curable sealing clear prime paint by roller coating, flow coating, or spray coating, to 10~150µm thickness.

Coat UV-curable glue: coat UV-curable sealing clear prime paint by roller coating, flow coating, or spray coating, to 2~150µm thickness.

Coat UV-curable metal prime paint: coat UV-curable metal prime paint by roller coating, flow coating, or spray coating, to 10~150µm thickness.

Transfer a transfer film: transfer a transfer film in a transfer machine.

Remove film: Remove the film with a manual or automatic film peeling machine.

Coat UV-curable protective varnish: coat UV-curable protective varnish by roller coating, flow coating, or spray coating, to 10~250µm thickness, at 10~100-degree adjustable glossiness (measured with a 60-degree glossmeter).

The UV-curable permeating agent, UV-curable paint filler, UV-curable sealing clear prime paint, UV-curable pigmented paint, UV-curable glue, UV-curable metal prime paint, and UV-curable protective varnish are paint or glue well known in the art. For example:
Calculated in weight percentage, the UV-curable permeating agent comprises 10-80% acrylate prepolymer, 10~89 % acrylate monomer, 1~5% photoinitiator, 0-2% auxiliary agent, and 0~50% solvent.
Calculated in weight percentage, the UV-curable paint filler comprises 10~80% acrylate prepolymer, 5~50 % acrylate monomer, 1~5% photoinitiator, 0~2% auxiliary agent, and 0~50% filler.
Calculated in weight percentage, the UV-curable sealing clear prime paint comprises 10~80% acrylate prepolymer, 5~60 % acrylate monomer, 1~6% photoinitiator, 0~2% auxiliary agent, and 0~50% filler.
Calculated in weight percentage, the UV-curable pigmented paint comprises 10-80% acrylate prepolymer, 5-60% acrylate monomer, 1-6% photoinitiator, 0~2% auxiliary agent, 0~50% filler, and 0~50% pigment.
Calculated in weight percentage, the UV-curable glue comprises 10~80% acrylate prepolymer, 5~60% acrylate monomer, 1~6% photoinitiator, 0~2% auxiliary agent, and 0~50% filler.
Calculated in weight percentage, the UV-curable metal prime paint comprises 10~80% acrylate prepolymer, 1~80% acrylate monomer, 1~15% photoinitiator, 0~5% auxiliary agent, and 0~30% filler.
Calculated in weight percentage, the UV-curable metal protective varnish usually comprises 10~80% acrylate prepolymer, 1~80% acrylate monomer, 1~15% photoinitiator, 0~5% auxiliary agent, 0~30% filler, and 0~30% solvent.

The acrylate prepolymer is the same as the acrylate prepolymer used to prepare the UV-curing transfer film or UV-curable colorful transfer film in the present invention. The photoinitiator is the same as the photoinitiator used to prepare the UV-curing transfer film or UV-curable colorful transfer film in the present invention.

The auxiliary agent is the same as the auxiliary agent used to prepare the UV-curing transfer film or UV-curable colorful transfer film in the present invention.

The filler can be any of talcum powder, calcium carbonate, and barium sulfate powder.

The solvent is selected from at least one compound in the group of methyl benzene, dimethyl benzene, ethyl acetate, butyl acetate, butanone, cyclohexanone, isopropanol, and ethylene glycol monobutyl ether.

UV-curing transfer films/UV-curable colorful transfer film decorative boards/plates obtained with the preparation method provided in the present invention have advantages such as high material strength, high weather resistance, environmental protection, rich colors and patterns, full and rigid paint film, high scratch resistance, fouling resistance and easy cleaning, and non-flammability, etc., and have better decorative and protective performance than existing thermal transfer films and aqueous transfer films.

The method for production of UV-curing transfer film provided in the present invention have advantages such as small equipment footprint, low equipment investment, high production efficiency, low energy consumption, and free of pollution, etc.; moreover, when the transfer film provided in the present invention is applied to timber boards, cement boards, gypsum boards, or metal plates, the transfer film adheres to the boards/plates firmly, and will not peel off from the boards/plates.

### Brief Description of the Drawings

Figure 1 is a sectional view of the structure of an UV-curing transfer film provided in the present invention;
Figure 2 is a sectional view of the structure of an UV-curing transfer film which is not according to the present invention.

### Brief Description of the Symbols in the Drawings

| | | |
|---|---|---|
| 1. substrate film, | 2. release agent layer, | 3. UV-curable protective layer |
| 4. UV-curable ink decorative pattern layer, | | 5. UV-curable paint background layer |

### Detailed Description of the Embodiments

### Embodiment 1: colorful transfer film with Arabescato Coccoha or Black Marquina marble texture

The structure of a colorful transfer film with Arabescato Coccoha or Black Marquina marble texture is shown in Figure 1. The colorful transfer film comprises a substrate film 1, a release agent layer 2, an UV-curable protective layer 3, an UV-curable ink decorative pattern layer 4, and an UV-curable paint background layer 5. The preparation method comprises the following steps:
1) Bake a polypropylene film (substrate film) at 120°C, to force the film to preshrink, and remove electrostatic charges.
2) Uniformly spread or print release agent on the surface of the polypropylene film prepared in step 1), and then cure the coating under infrared irradiation, i.e., adjust the infrared heating temperature to 60°C, let the coating to flow flat for 1 min., and cure the release agent completely, to obtain a release agent layer in 1 µm thickness.
   Calculated in weight percentage, the release agent is a mixture of 41 % methylol cellulose, 20% modified paraffin wax, 18% butanone, 5% ethyl acetate, 5% fluorine-containing amino acrylate, 10% butyl acrylate, and 1% 2-hydroxyl-2-methyl-1-phenyl-1-acetone.
3) Uniformly coat UV-curable protective paint on the surface of the release agent layer prepared in step 2) by spreading or printing, and then cure the UV-curable protective paint under UV irradiation as follows: convey a single layer of coiled material coated with the UV-curable protective paint through an UV curing machine equipped with 1~3 ultraviolet tubes (high-voltage mercury lamps) with 3~20Kw unit power and 0-3 metal halide lamps (iodine gallium lamps, iron lamps, or dysprosium lamps, etc.) with 3~20Kw unit power at a high speed, to cure the UV-curable protective paint under UV irradiation, and thereby obtain an UV-curable protective layer in 10µm thickness; the wavelength of the UV light source is 300~400nm, and the conveying speed of the UV curing machine is 1~200m/min.;
   Calculated in weight percentage, the UV-curable paint for the protective layer is:
   A. mixture of 20% fluorine-containing epoxy acrylate, 40% fluorine-containing polyurethane acrylate, 16% ethoxy- trimethylolpropane triacrylate (EO-TMPTA), 20% propoxy-trimethylolpropane triacrylate (PO-TMPTA), 3% 1-hydroxyl cyclohexyl phenyl ketone, 0.5% BYK 052, and 0.5% Disperbyk 103;
      Or
   B. Mixture of 10% fluorine-containing amino acrylate, 10% acrylate copolymer, 50% fluorine-containing acrylate copolymer, 9.5% hydroxyethyl methacrylate (HEMA), 10% trifluoro ethyl acrylate, 5% 1-hydroxyl cyclohexyl phenyl ketone, 0.2% BYK 052, 0.3% Disperbyk 103, and 5% GIFU matting agent (matting wax from Japan GIFU).
4) Uniformly coat black UV-curable ink or white UV-curable ink with patterns and decorative effect on the surface of the UV-curable protective layer prepared in step 3) by spreading or printing, and then cure the UV-curable ink under UV irradiation as follows: convey a single layer of coiled material coated with the black UV-curable ink or white UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the black UV-curable ink or white UV-curable ink under UV irradiation, and thereby obtain a black decorative pattern layer in 10µm thickness or white decorative pattern layer in 10µm thickness; the wavelength of the UV light source is 365~410nm, and the conveying speed of the UV curing machine is 1~200m/min.;
   Calculated in weight percentage, the black UV-curable ink for decorative pattern layer is a mixture of 18.5% fluorine-containing epoxy acrylate, 25% fluorine-containing polyurethane acrylate, 15% propoxy-neopentyl glycol diacrylate (PO-NPGDA), 15% phthalandione di-(diethylene glycol) diacrylate (PDDA), 3% 1-hydroxyl cyclohexyl phenyl ketone, 3% 2,4-diisopropyl thioxanthone, 0.2% BYK 052, 0.3% Disperbyk 103, 10% soot carbon M-E, and 10% polyamide resin;
   Calculated in weight percentage, the white UV-curable ink for decorative pattern layer is a mixture of 5% amino acrylate, 25% fluorine-containing amino acrylate, 5% acrylate copolymer, 10% tripropylene glycol diacrylate (TPGDA), 9.8% dipropylene glycol diacrylate (DPGDA), 2% 1-hydroxyl cyclohexyl phenyl ketone, 3% 2, 4, 6-trimethyl benzoyl diphenyl phosphine oxide (TPO), 0.1% BYK 052, 0.1% Disperbyk 103, 5% talcum powder, 25% titanium pigment, and 10% polyamide resin.
5) Uniformly coat white UV-curable ink on the surface of the black UV-curable decorative pattern layer or white UV-curable decorative pattern layer, and then cure the coating under UV irradiation as follows: convey a single layer of coil material coated with the white UV-curable ink through an UV curing machine equipped with 1-3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power, to cure the white UV-curable ink under UV irradiation, to obtain a colorful transfer film with Black Marquina marble texture or a colorful transfer film with Arabescato Coccoha marble texture, respectively;
   Calculated in weight percentage, the white UV-curable ink for background layer is: a mixture of 10% fluorine-containing epoxy acrylate, 25% fluorine-containing amino acrylate, 5% acrylate copolymer, 15% ethoxy- trimethylolpropane triacrylate (EO-TMPTA), 9.8% dipropylene glycol diacrylate (DPGDA), 3% 1-hydroxyl cyclohexyl phenyl ketone, 3% 2, 4, 6-trimethyl benzoyl diphenyl phosphine oxide (TPO), 0.2% BYK 052, 22% titanium pigment, and 7.2% polyamide resin.

### Embodiment 2. Colorful transfer film with Royal Batticino beige or buff texture

The structure of colorful transfer film with Royal Batticino beige or buff texture is the same as that in embodiment 1. The preparation method comprises the following steps:
1) Bake a polyethylene film (substrate film) at 160°C, to force the film to preshrink, and remove electrostatic charges.
2) Uniformly spread or print release agent on the surface of the polyethylene film prepared in step 1), and then cure the coating under infrared irradiation, i.e., adjust the infrared heating temperature to 150°C, let the coating to flow flat for 0.01min., and let the solvent in the coating to volatilize fully; cure the release agent completely, to obtain a release agent layer in 5µm thickness;
   Calculated in weight percentage, the release agent is a mixture of 30% methylol cellulose, 25% palm wax, 15% butanone, 5% ethyl acetate, 11% fluorine-containing polyurethane acrylate, 10% polyester acrylate, and 4% 1-hydroxyl cyclohexyl phenyl ketone.
3) Uniformly coat UV-curable protective paint on the surface of the release agent layer prepared in step 2) by spreading or printing, and then cure the UV-curable protective paint under UV irradiation as follows: convey a single layer of coiled material coated with the UV-curable protective paint through a TV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the UV-curable protective paint under UV irradiation, and thereby obtain an UV-curable protective layer in 15µm thickness; the wavelength of the UV light source is 250~380nm, and the conveying speed of the UV curing machine is 1~200m/min.;
   Calculated in weight percentage, the UV-curable paint for the protective layer is:
   A. mixture of 20% fluorine-containing epoxy acrylate, 40% fluorine-containing polyurethane acrylate, 10% ethoxy- trimethylolpropane triacrylate (EO-TMPTA), 20% propoxy-trimethylolpropane triacrylate (PO-TMPTA), 3% 1-hydroxyl cyclohexyl phenyl ketone, 0.5% BYK 052, 0.5% Disperbyk 103, and 6% butanone;
      Or
   B. mixture of 14% fluorine-containing amino acrylate, 10% acrylate copolymer, 50% fluorine-containing acrylate copolymer, 9.5% hydroxyethyl methacrylate (HEMA), 10% trifluoro ethyl acrylate, 2% 1-hydroxyl cyclohexyl phenyl ketone, 0.2% BYK 052, 0.3% BYK 358, and 4% GIFU matting agent (matting wax from Japan GIFU).
4) Uniformly coat beige UV-curable ink or buff UV-curable ink with patterns and decorative effect on the surface of the UV-curable protective layer prepared in step 3) by spreading or printing, and then cure the UV-curable ink under UV irradiation as follows: convey a single layer of coiled material coated with the beige UV-curable ink or buff UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the beige UV-curable ink or buff UV-curable ink under UV irradiation, and thereby obtain a beige decorative pattern layer in 15µm thickness or a buff decorative pattern layer in 18µm thickness; the wavelength of the UV light source is 300~420nm, and the conveying speed of the UV curing machine is 1~200m/min.;
   Calculated in weight percentage, the beige UV-curable ink for decorative pattern layer is:
   A mixture of 20% fluorine-containing acrylate copolymer, 20% fluorine-containing amino acrylate, 9.3% hydroxyethyl acrylate (HEA), 20% dipentaerythritol hexa-acrylate (DPHA), 2% 1-hydroxyl cyclohexyl phenyl ketone 2%, 3% 2-methyl-1-[4-(methyl sulfenyl)-phenyl]-2-morpholinyl-1-acetone, 0.2% BYK 052, 0.3% Disperbyk 103, 15% proflavin, 0.2% scarlet powder, and 10% vinyl chloride vinyl acetate;
   Calculated in weight percentage, the buff UV-curable ink for decorative pattern layer is: a mixture of 10% fluorine-containing epoxy acrylate, 20% fluorine-containing amino acrylate, 17.4% dipropylene glycol diacrylate (DPGDA), 20% dipentaerythritol hexa-acrylate (DPHA), 2% 2-hydroxyl-2-methyl-1-phenyl-1-acetone, 3% 2-methyl-1-[4-(methyl sulfenyl)-phenyl]-2-morpholinyl-1-acetone, 0.3% BYK 052, 0.3% Disperbyk 103, 2% proflavin, 20% titanium pigment, and 5% vinyl chloride vinyl acetate.
5) Uniformly coat white UV-curable ink on the surface of the beige UV-curable decorative pattern layer or buff UV-curable decorative pattern layer, and then cure the coating under UV irradiation as follows: convey a single layer of coil material coated with the white UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power, to cure the white UV-curable ink under UV irradiation, to obtain a colorful transfer film with Royal Batticino beige marble texture or a colorful transfer film with Royal Batticino buff marble texture, respectively.
   Calculated in weight percentage, the white UV-curable ink for background layer is:
   a mixture of 20% fluorine-containing epoxy acrylate, 25% ethoxy- trimethylolpropane triacrylate (EO-TMPTA), 2% 1-hydroxyl cyclohexyl phenyl ketone, 3% 2, 4, 6-trimethyl benzoyl diphenyl phosphine oxide, 2.9% butanone, 0.1% Disperbyk 103, 20% titanium pigment, and 27% polyamide resin.

### Embodiment 3 which is not according to the present invention: Colorful transfer film with timber texture

See Figure 2 for the structure of a colorful transfer film with timber texture. The colorful transfer film comprises a substrate film 1, a release agent layer 2, an UV-curable ink decorative pattern layer 4, and an UV-curable paint background layer 5. The preparation method comprises the following steps:
1) Bake a polyvinyl chloride film (substrate film) at 180°C, to force the film to preshrink, and remove electrostatic charges.
2) Uniformly spread or print release agent on the surface of the polyvinyl chloride film prepared in step 1), and then cure the coating under infrared irradiation, i.e., adjust the infrared heating temperature to 80 °C, let the coating to flow flat for 2min., and let the solvent in the coating to volatilize fully; cure the release agent completely, to obtain a release agent layer in 100µm thickness;
   Calculated in weight percentage, the release agent is a mixture of 30% methylol cellulose, 5% modified paraffin wax, 15% palm wax, 10% hydroxyl silicone oil, 11% butanone, 5% ethyl acetate, 12% fluorine-containing polyurethane acrylate, 10% trifluoro ethyl methacrylate, 0.5% 2-hydroxyl-2-methyl-1-phenyl-1-acetone, and 1.5% 1-hydroxyl cyclohexyl phenyl ketone.
3) Uniformly coat French gray UV-curable ink with patterns and decorative effect on the surface of the release agent layer prepared in step 2) by spreading or printing to obtain French gray timber grains, or uniformly coat red gray ink with patterns and decorative effect by spreading or coating to obtain red gray timber grains, and then cure the French gray UV-curable ink or red gray UV-curable ink under UV irradiation as follows: convey a single layer of coiled material coated with the French gray UV-curable ink or red gray UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the French gray UV-curable ink or red gray UV-curable ink under UV irradiation, and thereby obtain a French gray timber grain pattern layer in 10µm thickness or a red gray timber grain pattern layer in 10µm thickness, respectively; the wavelength of the UV light source is 250~420nm, and the conveying speed of the UV curing machine is 1~200m/min.;
   Calculated in weight percentage, the French gray UV-curable ink for decorative pattern layer is:
   a mixture of 23% fluorine-containing polyurethane acrylate, 15% polyester acrylate, 10.4% dipentaerythritol hexa-acrylate (DPHA), 15% 1, 6-ethylene glycol diacrylate (HDDA), 2% 2-hydroxyl-2-methyl-1-phenyl-1-acetone, 3% 3% 2, 4, 6-trimethyl benzoyl diphenyl phosphine oxide, 0.2% BYK 052, 0.3% Disperbyk 103, 0.1% soot carbon, 20% titanium pigment, 4% vinyl chloride vinyl acetate, 5% polyamide resin, and 2% butanone.
   Calculated in weight percentage, the red gray UV-curable ink for decorative pattern layer is:
      a mixture of 10% fluorine-containing epoxy acrylate, 23% fluorine-containing polyurethane acrylate, 12% dipropylene glycol diacrylate (DPGDA), 2% 1-hydroxyl cyclohexyl phenyl ketone, 3% 2, 4, 6-trimethyl benzoyl diphenyl phosphine oxide 3%, 0.3% BYK 052, 0.1% Disperbyk 103, 1% scarlet powder, 0.1% soot carbon, 21% titanium pigment, 3% calcium carbonate, 10% polyamide resin, 4.5% butanone, and 10% ethyl acetate.
5) Uniformly coat white UV-curable ink on the surface of the French gray timber grain pattern layer or red gray timber grain pattern layer prepared in step 3), and then cure the coating under UV irradiation as follows: convey a single layer of coil material coated with the white UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power, to cure the white UV-curable ink under UV irradiation, to obtain a colorful transfer film with French gray timber texture or a colorful transfer film with red gray timber texture, respectively.
   Calculated in weight percentage, the white UV-curable ink for background layer is:
   a mixture of 10% fluorine-containing epoxy acrylate, 17.5% fluorine-containing amino acrylate, 10% acrylate copolymer, 10% ethoxy- trimethylolpropane triacrylate (EO-TMPTA), 10% dipropylene glycol diacrylate (DPGDA), 2% 2-hydroxyl-2-methyl-1-phenyl-1-acetone, 3% 2, 4, 6-trimethyl benzoyl diphenyl phosphine oxide, 0.2% BYK 052, 25% titanium pigment, 10% thermoplastic acrylic, and 2.3% ethyl acetate.

### Embodiment 4: Colorful transfer film with red crystal diamond effect

The structure of a colorful transfer film with red crystal diamond effect is the same as that in embodiment 1. The preparation method comprises the following steps:
1) Bake a polyethylene terephthalate film (substrate film) at 60°C, to force the film to preshrink and remove electrostatic charges.
2) Uniformly spread or print release agent on the surface of the polyethylene terephthalate film prepared in step 1), and then cure the coating under infrared irradiation, i.e., adjust the infrared heating temperature to 90°C, let the coating to flow flat for 1 min., and let the solvent in the coating to volatilize fully; cure the release agent completely, to obtain a release agent layer in 10µm thickness;
   Calculated in weight percentage, the release agent is a mixture of 20% methylol cellulose, 10% modified paraffin wax, 9% phenylmethyl silicone oil, 20% butanone, 15% ethyl acetate, 20% fluorine-containing polyester acrylate, 5% PO-NPGDA, 0.5% 2-hydroxyl-2-methyl-1-phenyl-1-acetone, and 0.5% 1-hydroxyl cyclohexyl phenyl ketone.
3) Uniformly coat UV-curable protective paint on the surface of the release agent layer prepared in step 2) by spreading or printing, and then cure the UV-curable protective paint under UV irradiation as follows: convey a single layer of coiled material coated with the UV-curable protective paint through a TV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the UV-curable protective paint under UV irradiation, and thereby obtain an UV-curable protective layer in 15µm thickness; the wavelength of the UV light source is 285~400nm, and the conveying speed of the UV curing machine is 1~200m/min.;
   Calculated in weight percentage, the UV-curable paint for the protective layer is:
   A. mixture of 10% fluorine-containing epoxy acrylate, 34.3% fluorine-containing amino acrylate, 30% hexafluoro butyl methacrylate, 20% dodecafluoro heptyl methacrylate, 3% 2-hydroxyl-2-methyl-1-phenyl-1-acetone, 2% 1-hydroxyl cyclohexyl phenyl ketone, 0.2% BYK 052, and 0.5% Disperbyk 103;
      Or
   B. mixture of 10% fluorine-containing amino acrylate, 50% fluorine-containing acrylate copolymer, 17.8% trifluoro ethyl methacrylate, 10% ethoxy- trimethylolpropane triacrylate (EO-TMPTA), 2% 2-hydroxyl-2-methyl-1-phenyl-1-acetone, 3% 1-hydroxyl cyclohexyl phenyl ketone, 0.1% BYK 052, 0.1% Disperbyk 103, and 7% GIFU matting agent (matting wax from Japan GIFU).
4) Uniformly coat pearlescent UV-curable ink or clear red UV-curable ink with patterns and decorative effect on the surface of the UV-curable protective layer prepared in step 3) by spreading or printing, and then cure the UV-curable ink under UV irradiation as follows: convey a single layer of coiled material coated with the pearlescent UV-curable ink or clear red UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the pearlescent UV-curable ink or clear red UV-curable ink under UV irradiation, and thereby obtain a pearlescent ink decorative pattern layer in 20µm thickness or a clear red ink decorative pattern layer in 20µm thickness, respectively; the wavelength of the UV light source is 300~420nm, and the conveying speed of the UV curing machine is 1~200m/min.;
   Calculated in weight percentage, the pearlescent UV-curable ink for decorative pattern layer is a mixture of 15% fluorine-containing polyurethane acrylate, 15% amino acrylate, 15% hexafluoro butyl acrylate, 20% dodecafluoro heptyl acrylate, 2% 2-hydroxyl-2-methyl-1-phenyl-1-acetone, 2.7% 2, 4, 6-trimethyl benzoyl diphenyl phosphine oxide, 0.2% BYK 052, 0.1% Disperbyk 103, 20% pearl essence, and 10% polyamide resin.
   Calculated in weight percentage, the clear red UV-curable ink for decorative pattern layer is a mixture of 12% acrylate copolymer, 12.4% fluorine-containing polyurethane acrylate, 10% polyester acrylate, 10% ethylhexyl acrylate (EHA), 15% ethoxy-trimethylolpropane triacrylate (EO-TMPTA), 10% methacrylic acid, 2% 1-hydroxyl cyclohexyl phenyl ketone 3% 2, 4, 6-trimethyl benzoyl diphenyl phosphine oxide, 0.3% BYK 052, 5% clear iron oxide red, and 20.3% polyamide resin.
5) Uniformly coat white UV-curable ink on the surface of the pearlescent UV-curable decorative pattern layer or clear red UV-curable decorative pattern layer, and then cure the coating under UV irradiation as follows: convey a single layer of coil material coated with the white UV-curable ink through an UV curing machine equipped with 1~3 ultraviolet tubes (high-voltage mercury lamps) with 3~20Kw unit power and 0-3 metal halide lamps (iodine gallium lamps, iron lamps, or dysprosium lamps, etc.) with 3~20Kw unit power, to cure the white UV-curable ink under UV irradiation, to obtain a pearlescent transfer film with red crystal diamond effect or a clear red transfer film with red crystal diamond effect, respectively.
   Calculated in weight percentage, the white UV-curable ink for background layer is:
   a mixture of 15% fluorine-containing epoxy acrylate, 32% ethoxy- trimethylolpropane triacrylate (EO-TMPTA), 5% dipropylene glycol diacrylate, 2% 1-hydroxy cyclohexyl phenyl ketone, 3% 2, 4, 6-trimethyl benzoyl diphenyl phosphine oxide, 20% titanium pigment, 5% talcum powder, and 18% polyamide resin.

### Embodiment 5. Colorful transfer film with poetry images

The structure of a colorful transfer film with poetry images is the same as that in embodiment 1. The preparation method comprises the following steps:
1) Bake a polyvinyl chloride film (substrate film) at 140°C, to force the film to preshrink, and remove electrostatic charges.
2) Uniformly spread or print release agent on the surface of the polyvinyl chloride film prepared in step 1), and then cure the coating under infrared irradiation, i.e., adjust the infrared heating temperature to 120°C, let the coating to flow flat for 0.5min., and let the solvent in the coating to volatilize fully; cure the release agent completely, to obtain a release agent layer in 20µm thickness;
   Calculated in weight percentage, the release agent is a mixture of 33% methylol cellulose, 5% modified paraffin wax, 15% palm wax, 2% methyl-silicone oil, 3% phenylmethyl silicone oil, 20% butanone, 5% ethyl acetate, 5% fluorine-containing amino acrylate, 10% dipropylene glycol diacrylate (DPGDA), and 2% 2-hydroxyl-2-methyl-1-phenyl-1-acetone.
3) Uniformly coat UV-curable protective paint on the surface of the release agent layer prepared in step 2) by spreading or printing, and then cure the UV-curable protective paint under UV irradiation as follows: convey a single layer of coiled material coated with the UV-curable protective paint through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the UV-curable protective paint under UV irradiation, and thereby obtain an UV-curable protective layer in 15µm thickness; the wavelength of the UV light source is 200~380nm, and the conveying speed of the UV curing machine is 1~200m/min.;
   Calculated in weight percentage, the UV-curable paint for the protective layer is:
   A. mixture of 30% fluorine-containing polyester acrylate, 30% fluorine-containing polyurethane acrylate, 16% trifluoro ethyl methacrylate, 18.5% propoxy-trimethylolpropane triacrylate (PO-TMPTA), 3% 2-hydroxyl-2-methyl-1-phenyl-1-acetone, 0.1% BYK 052, 2% talcum powder, and 0.4% ethyl acetate;
      Or
   B. mixture of fluorine-containing amino acrylate 20%, 10% polyurethane acrylate, 30% fluorine-containing acrylate copolymer, 14% ethoxy-trimethylolpropane triacrylate (EO-TMPTA), 10% trifluoro ethyl acrylate, 5% 1-hydroxyl cyclohexyl phenyl ketone, 0.4% talcum powder, 0.6% ethyl acetate, and 10% matting powder.
4) Uniformly coat mirror silver UV-curable ink or mirror gold UV-curable ink with patterns and decorative effect on the surface of the UV-curable protective layer prepared in step 3) by spreading or printing, and then cure the UV-curable ink under UV irradiation as follows: convey a single layer of coiled material coated with the mirror silver UV-curable ink or mirror gold UV-curable ink through an UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power at a high speed, to cure the mirror silver UV-curable ink or mirror gold UV-curable ink under UV irradiation, and thereby obtain a mirror silver decorative pattern layer in 25µm thickness or a mirror gold decorative pattern layer in 25µm thickness, respectively; the wavelength of the UV light source is 250~400nm, and the conveying speed of the UV curing machine is 1~200m/min.;
   Calculated in weight percentage, the mirror silver UV-curable ink for decorative pattern layer is:
   a mixture of 14.5% fluorine-containing polyurethane acrylate, 15% fluorine-containing epoxy acrylate, 15% hexafluoro butyl acrylate, 15% hexafluoro butyl methacrylate, 2% 2-hydroxyl-2-methyl-1-phenyl-1-acetone, 3% 2, 4, 6-trimethyl benzoyl diphenyl phosphine oxide, 0.2% BYK 052, 0.3% butanone, 15% silver powder, and 20% thermoplastic acrylic.
   Calculated in weight percentage, the mirror gold UV-curable ink for decorative pattern layer is:
      a mixture of 15% fluorine-containing acrylate copolymer, 16.1% amino acrylate, 15% dipentaerythritol hexa-acrylate (DPHA), 2% 1-hydroxyl cyclohexyl phenyl ketone, 2% 2, 4, 6-trimethyl benzoyl diphenyl phosphine oxide, 0.2% BYK 052, 0.2% Disperbyk 103, 18% gold powder, 10% polyamide resin, and 1.5% thermoplastic acrylic.
5) Uniformly coat black UV-curable ink on the surface of the mirror silver UV-curable decorative pattern layer or mirror gold UV-curable decorative pattern layer, and then cure the coating under UV irradiation as follows: convey a single layer of coil material coated with the black UV-curable ink through a UV curing machine equipped with 1~3 ultraviolet tubes (high-voltage mercury lamps) with 3~20Kw unit power and 0~3 metal halide lamps (iodine gallium lamps, iron lamps, or dysprosium lamps, etc.) with 3~20Kw unit power, to cure the black UV-curable ink under UV irradiation, to obtain a mirror silver colorful transfer film with poetry images or a mirror gold colorful transfer film with poetry images, respectively.
   Calculated in weight percentage, the black UV-curable ink for background layer is:
   a mixture of 15% fluorine-containing polyester acrylate, 27.7% fluorine-containing amino acrylate, 7% trifluoro ethyl methacrylate, 20% dipropylene glycol diacrylate (DPGDA), 2% 1-hydroxyl cyclohexyl phenyl ketone, 3% 2, 4-diisopropyl thioxanthone, 0.1% BYK 052, 0.2% Disperbyk 103, 8% soot carbon, 2% talcum powder, and 15% polyamide resin.

### Embodiment 6. Decorative board with marble texture

The substrate of the decorative board is a fiber reinforced cement board, fiber reinforced calcium silicate board, fiber reinforced magnesium oxide board, light-weight magnesium chloride cement board, magnesium oxychloride board, or gypsum board; first, treat the substrate by sanding and remove dust from the surface; then, brush a layer of UV-curable permeating agent on the surface of the substrate at a 120g/m2 coating rate, and then hold for 30min. to let the coating to flow flat naturally; next, coat a layer of UV-curable paint filler in thickness of 20µm by roller coating; load the coated substrate into an UV curing machine that is equipped with a 9.6Kw UV lamp (high-voltage mercury lamp) and operates at 15m/min. conveying speed to cure the coating; then, coat a layer of UV-curable sealing clear prime paint in thickness of 40µm on the surface of the UV-curable paint filler; load the coated board into an UV curing machine that is equipped with two 13Kw UV lamps (high-voltage mercury lamps) and operates at 15m/min. conveying speed to cure the coating; next, treat the board by sanding on a sanding machine, with a 240-mesh abrasive belt, and remove dust from the surface of the board; then, coat a layer of UV-curable sealing clear prime paint in thickness of 10µm on the surface of the existing UV-curable sealing clear prime paint by roller coating; load the coated board into an UV curing machine that is equipped with a 9.6KW UV lamp (high-voltage mercury lamp) and operates at 15m/min. conveying speed to cure the coating; next, coat a layer of white UV-curable prime paint in thickness of 10µm on the surface of the UV-curable sealing clear prime paint; load the coated board into an UV curing machine that is equipped with five 16.8Kw UV lamps (metal halide lamps) and operates at 15m/min. conveying speed to cure the coating; then, treat the board by sanding on a sanding machine, with a 400-mesh abrasive belt; next, coat a layer of UV-curable glue in thickness of 10µm on the surface of the white UV-curable prime paint, and then transfer a colorful transfer film with Black Marquina marble texture or a colorful transfer film with Arabescato Coccoha marble texture as described in embodiment 1 onto the surface of the UV-curable glue; load the coated board into an UV curing machine that is equipped with six 16.8Kw UV lamps (metal halide lamps) and operates at 15m/min. conveying speed to cure the coating; then, remove the film, and let the coating to flow flat for 2min. under infrared irradiation at 90°C temperature; next, load the coated board into an UV curing machine that is equipped with three 13Kw UV lamps (high-voltage mercury lamps) and operates at 15m/min. conveying speed to cure the coating; next, after the treated board is inspected as acceptable, apply a polypropylene protective film on the surface of the board, to obtain a finished decorative board with marble texture finally.

Calculated in weight percentage, the UV-curable permeating agent comprises: 20% epoxy acrylate, 50% TMPTA, 10% TPGDA, 4% 2-hydroxyl-2-methyl-1-phenyl-1-acetone, and 16% ethyl acetate.

Calculated in weight percentage, the UV-curable paint filler comprises: 40% epoxy acrylate, 20% polyester acrylate, 16% TMPTA, 20% talcum powder, 3.5% 2-hydroxyl-2-methyl-1-phenyl-1-acetone, 0.2% BYK 052, and 0.3% Disperbyk 163.

Calculated in weight percentage, the UV-curable sealing clear prime paint comprises: 20% fluorine-containing epoxy acrylate, 30% polyurethane acrylate, 10% TPGDA, 20% EO-TMPTA, 15% talcum powder, 4.5% hydroxyl cyclohexyl phenyl ketone, 0.2% BYK 055, and 0.3% Disperbyk 103.

Calculated in weight percentage, the UV-curable white prime paint comprises: 20% epoxy acrylate, 30% fluorine-containing polyester acrylate, 20% PETA, 10% PO-NPGDA, 15% titanium pigment, 2% 1-hydroxyl cyclohexyl phenyl ketone, 2.5% 2, 4, 6-trimethyl benzoyl diphenyl phosphine oxide, 0.2% BYK 052, and 0.3% Disperbyk 103.

Calculated in weight percentage, the UV-curable glue comprises: 35% polyurethane acrylate, 30% fluorine-containing polyester acrylate, 20% PETA, 10% PO-NPGDA, 2.5% 1-hydroxyl cyclohexyl phenyl ketone, 2% 2-hydroxyl-2-methyl-1-phenyl-1-acetone, 0.2% BYK 052, and 0.3% Disperbyk 103.

### Embodiment 7 which is not according to the present invention: Decorative board with timber texture

The substrate of the decorative board is a solid timber board, MDF board, or plywood board; first, treat the substrate by sanding and remove dust from the surface; then, coat a layer of UV-curable sealing prime paint in thickness of 40µm on the surface of the substrate; load the coated board into an HV curing machine that is equipped with two 9.6Kw UV lamps (high-voltage mercury lamps) and operates at 8m/min. conveying speed to cure the coating; then, treat the board by sanding and remove dust from the surface, and coat a layer of UV-curable glue in thickness of 10µm on the surface of the UV-curable sealing prime paint; next, cure the UV-curable glue, and then transfer a colorful transfer film with timber texture (French gray grains) and a colorful transfer film with timber texture (red gray longitudinal grains) as described in embodiment 3; load the transfer film with timber texture into an UV curing machine that is equipped with three 16.8Kw UV lamps (metal halide lamps) and operates at 8m/min. conveying speed to cure the coating; next, remove the film, and let the coating to flow flat for 2min. under infrared irradiation at 90°C temperature; next, coat a layer of UV-curable in thickness of 10µm on the surface of the transfer film, cure the glue, and then coat a layer of UV-curable protective semi-matt varnish in thickness of 20µm at 60-degree glossiness (measured with a 60-degree glossmeter) by roller coating; let the coating to flow flat for 1min. under infrared irradiation at 50°C temperature; load the coated board into an UV curing machine that is equipped with three 16.8KW UV lamps (metal halide lamps) and operates at 8m/min. conveying speed to cure the coating; after the decorative board is inspected as acceptable, apply a polypropylene protective film on the surface, to obtain a finished decorative board with timber texture finally.

Calculated in weight percentage, the UV-curable sealing prime paint comprises: 10% epoxy acrylate, 40% polyurethane acrylate, 20% EO-TMPTA, 10% PO-NPGDA, 15% talcum powder, 4.5% 1-hydroxy cyclohexyl phenyl ketone, 0.2% BYK 052, and 0.3% Disperbyk 103.

Calculated in weight percentage, the UV-curable glue comprises: 35% polyurethane acrylate, 30% fluorine-containing polyester acrylate, 20% PETA, 10% PO-NPGDA, 4.5% 1-hydroxyl cyclohexyl phenyl ketone, 0.2% BYK 052, and 0.3% Disperbyk 103. calculated in weight percentage, the UV-curable semi-matt protective varnish comprises: 30% polyurethane acrylate, 30% fluorine-containing polyurethane acrylate, 10% acrylate copolymer, 10% TMPTA, 10% PETA, 4% 1-hydroxyl cyclohexyl phenyl ketone, 5% matting powder, 0.2% BYK 055, 0.3% BYK 306, and 0.5% Disperbyk 103.

### Embodiment 8. Decorative plate with red crystal diamond effect

The substrate of the decorative plate is an aluminum plate, steel plate, or iron plate; first, clean up the substrate, remove oil stains, foreign matters, and dust from the surface of the substrate; then, coat a layer of UV-curable metal prime paint in thickness, of 10µm on the surface of the substrate by roller coating; load the coated substrate into an UV curing machine that is equipped with three 13Kw UV lamps (high-voltage mercury lamps) and operates at 10m/min. conveying speed to cure the paint; next, coat a layer of UV-curable glue in thickness of 10µm on the surface of the UV-curable metal prime paint, cure the glue, and then transfer a colorful transfer film with red crystal diamond effect as described in embodiment 4 onto the surface of the UV-curable glue; load the plate into an UV curing machine that is equipped with three 16.8Kw UV lamps (metal halide lamps) and operates at 10m/min. conveying speed to cure the coating; remove the film, and let the coating to flow flat for 2min. under infrared irradiation at 90°C temperature; next, load the plate into an UV curing machine that is equipped with four 16.8KW UV lamps (metal halide lamps) and operates at 10m/min. conveying speed to cure the coating completely; after the plate is inspected as acceptable, apply a polypropylene protective film on the surface, to obtain a finished product decorative plate with red crystal diamond effect finally.

Calculated in weight percentage, the UV-curable metal prime paint comprises: 15% epoxy acrylate, 35% polyurethane acrylate, 20% TMPTA, 10% PO-NPGDA, 15% talcum powder, 4.5% 1-hydroxyl cyclohexyl phenyl ketone, 0.2% BYK 052, and 0.3% Disperbyk 103.

Calculated in weight percentage, the UV-curable glue comprises: 35% polyurethane acrylate, 30% fluorine-containing polyester acrylate, 20% PETA, 10% PO-NPGDA, 4.5% 1-hydroxyl cyclohexyl phenyl ketone, 0.2% BYK 052, and 0.3% Disperbyk 103.

## Claims

1. A UV-curing transfer film, comprising a substrate film (1), a release agent layer (2), a UV-curing paint protective layer (3), a UV-curing ink decorative pattern layer (4), and a UV-curing paint background layer (5), the release agent layer (2) being on the substrate film (1), the UV-curing paint protective layer (3) being on the release agent layer (2), the UV-curing ink decorative pattern layer (4) being on the UV-curing paint protective layer (3), and the UV-curing paint background layer (5) is on the UV-curing ink decorative pattern layer (4);
wherein:
the substrate film (1) is any of polypropylene film, polyethylene film, polyvinyl chloride film, and polyethylene terephthalate film;
the release agent layer (2) is formed by a release agent which is a mixture of 20~50wt% cellulose, 1~30wt% wax, 0~10wt% silicone oil, 0~20wt% butanone, 0~15wt% ethyl acetate, 5~20wt% acrylate prepolymer, 5~20wt% acrylate monomer, and 1~6wt% photoinitiator;
the UV-curing paint protective layer (3) is formed by a UV-curable paint which is a mixture of 10~80wt% acrylate prepolymer, 5~50wt% acrylate monomer, 1~6wt% photoinitiator, 0~2wt% auxiliary agent, 0~50wt% filler, 0~10wt% butanone, and 0~15wt% ethyl acetate; or
a mixture of 10~80wt% acrylate prepolymer, 5~50wt% acrylate monomer, 1~6wt% photoinitiator, 0~2wt% auxiliary agent, 0~50wt% filler, 1~50wt% matting agent, 0~10wt% butanone, and 0~15wt% ethyl acetate;
the UV-curing ink decorative pattern layer (4) is formed by a UV-curable ink which is a mixture of 10~60wt% acrylate prepolymer, 5~50wt% acrylate monomer, 1~5wt% photoinitiator, 0~2wt% auxiliary agent, 0~50wt% filler, 5~30wt% toner, 5~30wt% resin, 0~10wt% butanone, and 0~15wt% ethyl acetate; and
the UV-curing paint background layer (5) is formed by a UV-curable paint which is a mixture of 10~50wt% acrylate prepolymer, 10~40wt% acrylate monomer, 1~5wt% photoinitiator, 0~2wt% auxiliary agent, 0~30wt% filler, 5~30wt% toner, 5~50wt% resin, 0~10wt% butanone, and 0~15wt% ethyl acetate.

2. The UV-curing transfer film according to claim 1, wherein:
the cellulose is methylol cellulose;
the wax is modified paraffin wax, palm wax, a mixture of them;
the silicone oil is at least one selected from methyl-silicone oil, benzyl silicone oil, and hydroxyl silicone oil.

3. The UV-curing transfer film according to claim 1 or 2, wherein: the polypropylene film is a modified polypropylene film.

4. The UV-curing transfer film according to any one of claims 1 to 3, wherein:
the acrylate prepolymer is at least one selected from epoxy acrylate, fluorine-containing epoxy acrylate, polyurethane acrylate, fluorine-containing polyurethane acrylate, polyester acrylate, fluorine-containing polyester acrylate, amino acrylate, fluorine-containing amino acrylate, acrylate copolymer, and fluorine-containing acrylate copolymer;
the acrylate monomer is at least one selected from butyl acrylate, cyclohexyl acrylate, ethylhexyl acrylate, hydroxyethyl acrylate, hydroxyethyl methacrylate, trifluoro ethyl acrylate, trifluoro ethyl methacrylate, hexafluoro butyl acrylate, hexafluoro butyl methacrylate, dodecafluoro heptyl acrylate, dodecafluoro heptyl methacrylate, tripropylene glycol diacrylate, dipropylene glycol diacrylate, neopentyl glycol diacrylate, propoxy-neopentyl glycol diacrylate, phthalandione di-(diethylene glycol) diacrylate, 1,6-hexylene glycol diacrylate, trimethylolpropane triacrylate, ethoxy-trimethylolpropane triacrylate, propoxy-trimethylolpropane triacrylate, pentaerythritol triacrylate, and dipentaerythritol hexa-acrylate;
the photoinitiator is at least one selected from benzoin ether photoinitiator, benzil ketal photoinitiator, acetophenone photoinitiator, anthraquinone photoinitiator, thioxanthone photoinitiator, benzophenone photoinitiator, acyl phosphine oxide photoinitiator, and benzoate photoinitiator,
the resin is at least one selected from modified polyvinyl acetate, polyamide resin, and thermoplastic acrylic;
the toner is at least one selected from soot carbon, titanium pigment, phthalocyanine blue, proflavine, and scarlet powder,
the auxiliary agent is at least one selected from leveling agent, anti-foaming agent, and wetting and dispersing agent;
the filler is at least one selected from talcum powder, calcium carbonate, and barium sulfate;
the matting agent is matting wax, matting powder, or a mixture of them.

5. The UV-curing transfer film according to claim 4, wherein: the modified polyvinyl acetate is vinyl chloride vinyl acetate, ethylene vinyl acetate, or a mixture of them.

6. The UV-curing transfer film according to claim 4, wherein:
the benzoin ether photoinitiator is at least one selected from benzoin methyl ether, benzoin ethyl ether, and benzoin isopropyl ether;
the benzil ketal photoinitiator is benzil dimethyl ketal;
the acetophenone photoinitiator is at least one selected from acetophenone, 2,2-di-methoxy-2-phenyl acetophenone, 2,2-diethoxy-2-phenyl acetophenone, 1,1-dichloro-acetophenone, 1-hydroxyl acetophenone, 1-hydroxyl cyclohexyl phenyl ketone, 2-hydroxyl-2-methyl-1-phenyl-1-acetone, 1-(4-isopropyl phenyl)-2-hydroxyl-2-methyl-1-acetone, 1-[4-(2-hydroxyl ethyoxyl) phenyl]-2-hydroxyl-2-methyl-1-acetone, 2-methyl-1-[4-(methyl sulfenyl) phenyl]-2-morpholinyl-1-acetone, and 2-benzyl-2-dimethyl amido-1-(4-morpholinyl phenyl)-1-butanone;
the anthraquinone photoinitiator is at least one selected from 2-tertiary butyl anthraquinone, 1-chlorine anthraquinone, and 2-amyl anthraquinone;
the thioxanthone photoinitiator is at least one selected from 2, 4-dimethyl thioxanthone, 2, 4-dimethyl thioxanthone, 2-isopropyl thioxanthone, 4-isopropyl thioxanthone, 2-chloro-thioxanthone, and 2, 4-diisopropyl thioxanthone;
the benzophenone photoinitiator is at least one selected from diphenyl ketone, 4-chlorine diphenyl ketone, methyl benzophenone, and 4-benzoyl-4'-methyl diphenyl thioether;
the acyl phosphine oxide photoinitiator is at least one selected from 2, 4, 6-trimethyl benzoyl diphenyl phosphine oxide, di-(2, 4, 6-trimethyl benzoyl)-phenyl phosphine oxide, di-(2, 6-dimethyl benzoyl)-2, 4, 4-trimethyl amyl phosphine oxide, and 2, 4, 6-trimethyl benzoyl phenyl ethyoxyl phosphine oxide;
the benzoate photoinitiator is methyl benzoylbenzoate, methyl ortho-benzoylbenzoate, or a mixture of them.

7. A method for preparation of the UV-curing transfer film according to any of claims 1 to 6, including: uniformly coating or printing a release agent on a substrate film (1), and then curing the release agent by infrared irradiation, to obtain a release agent layer (2) on the substrate film (1); uniformly coating or printing UV-curable protective paint on the release agent layer (2), and then curing the paint by UV irradiation, to obtain a UV-curing paint protective layer (3); uniformly coating or printing UV-curable ink that has patterns and decorative effect on the UV-curing paint protective layer (3), and then curing the ink by UV irradiation, to obtain an UV-curing ink decorative pattern layer (4); and uniformly coating or printing UV-curable background paint on the UV-curing ink decorative pattern layer (4), and then curing the paint by UV irradiation, to obtain the UV-curing transfer film, wherein:
the substrate film (1) is any of polypropylene film, polyethylene film, polyvinyl chloride film, and polyethylene terephthalate film;
the release agent layer (2) is formed by a release agent which is a mixture of 20~50wt% cellulose, 1~30wt% wax, 0~10wt% silicone oil, 0~20wt% butanone, 0~15wt% ethyl acetate, 5~20wt% acrylate prepolymer, 5~20wt% acrylate monomer, and 1~6wt% photoinitiator;
the UV-curing paint protective layer (3) is formed by a UV-curable paint which is a mixture of 10~80wt% acrylate prepolymer, 5~50wt% acrylate monomer, 1~6wt% photoinitiator, 0~2wt% auxiliary agent, 0~50wt% filler, 0~10wt% butanone, and 0~15wt% ethyl acetate; or a mixture of 10~80wt% acrylate prepolymer, 5~50wt% acrylate monomer, 1~6wt% photoinitiator, 0~2wt% auxiliary agent, 0~50wt% filler, 1~50wt% matting agent, 0~10wt% butanone, and 0~15wt% ethyl acetate;
the UV-curing ink decorative pattern layer (4) is formed by a UV-curable ink which is a mixture of 10~60wt% acrylate prepolymer, 5~50wt% acrylate monomer, 1~5wt% photoinitiator, 0~2wt% auxiliary agent, 0~50wt% filler, 5~30wt% toner, 5~30wt% resin, 0~10wt% butanone, and 0~15wt% ethyl acetate;
the UV-curing paint background layer (5) is formed by a UV-curable paint which is a mixture of 10~50wt% acrylate prepolymer, 10~40wt% acrylate monomer, 1~5wt% photoinitiator, 0~2wt% auxiliary agent, 0~30wt% filler, 5~30wt% toner, 5~50wt% resin, 0~10wt% butanone, and 0~15wt% ethyl acetate.

8. The method according to claim 7, wherein:
the cellulose is methylol cellulose;
the wax is modified paraffin wax, palm wax, a mixture of them;
the silicone oil is at least one selected from methyl-silicone oil, benzyl silicone oil, and hydroxyl silicone oil.

9. The method according to claims 7 or 8, wherein: the polypropylene film is a modified polypropylene film.

10. The method according to any of claims 7 to 9, wherein:
the acrylate prepolymer is at least one selected from epoxy acrylate, fluorine-containing epoxy acrylate, polyurethane acrylate, fluorine-containing polyurethane acrylate, polyester acrylate, fluorine-containing polyester acrylate, amino acrylate, fluorine-containing amino acrylate, acrylate copolymer, and fluorine-containing acrylate copolymer;
the acrylate monomer is at least one selected from butyl acrylate, cyclohexyl acrylate, ethylhexyl acrylate, hydroxyethyl acrylate, hydroxyethyl methacrylate, trifluoro ethyl acrylate, trifluoro ethyl methacrylate, hexafluoro butyl acrylate, hexafluoro butyl methacrylate, dodecafluoro heptyl acrylate, dodecafluoro heptyl methacrylate, tripropylene glycol diacrylate, dipropylene glycol diacrylate, neopentyl glycol diacrylate, propoxy-neopentyl glycol diacrylate, phthalandione di-(diethylene glycol) diacrylate, 1,6-hexylene glycol diacrylate, trimethylolpropane triacrylate, ethoxy-trimethylolpropane triacrylate, propoxy-trimethylolpropane triacrylate; pentaerythritol triacrylate, and dipentaerythritol hexa-acrylate;
the photoinitiator is at least one selected from benzoin ether photoinitiator, benzil ketal photoinitiator, acetophenone photoinitiator, anthraquinone photoinitiator, thioxanthone, photoinitiator, benzophenone photoinitiator, acyl phosphine oxide photoinitiator, and benzoate photoinitiator,
the resin is at least one selected from modified polyvinyl acetate, polyamide resin, and thermoplastic acrylic;
the toner is at least one selected from soot carbon, titanium pigment, phthalocyanine blue, proflavine, and scarlet powder,
the auxiliary agent is at least one selected from leveling agent, anti-foaming agent, and wetting and dispersing agent;
the filler is at least one selected from talcum powder, calcium carbonate, and barium sulfate; the matting agent is matting wax, matting powder, or a mixture of them.

11. The method according to claim 10, wherein: the modified polyvinyl acetate is vinyl chloride vinyl acetate, ethylene vinyl acetate, or a mixture of them.

12. The method according to any of claims 10 to 11, wherein: the benzoin ether photoinitiator is at least one selected from benzoin methyl ether, benzoin ethyl ether, and benzoin isopropyl ether;
the benzil ketal photoinitiator is benzil dimethyl ketal;
the acetophenone photoinitiator is at least one selected from acetophenone, 2,2-di-methoxy-2-phenyl acetophenone, 2,2-diethoxy-2-phenyl acetophenone, 1,1-dichloro-acetophenone, 1-hydroxyl acetophenone, 1-hydroxyl cyclohexyl phenyl ketone, 2-hydroxyl-2-methyl-1-phenyl-1-acetone, 1-(4-isopropyl phenyl)-2-hydroxyl-2-methyl-1-acetone, 1-(4-(2-hydroxyl ethyoxyl) phenyl]-2-hydroxyl-2-methyl-1-acetone, 2-methyl-1-[4-(methyl sulfenyl) phenyl]-2-morpholinyl-1-acetone, and 2-benzyl-2-dimethyl amido-1-(4-morpholinyl phenyl)-1-butanone;
the anthraquinone photoinitiator is at least one selected from 2-tertiary butyl anthraquinone, 1-chlorine anthraquinone, and 2-amyl anthraquinone;
the thioxanthone photoinitiator is at least one selected from 2, 4-dimethyl thioxanthone, 2, 4-diethyl thioxanthone, 2-isopropyl thioxanthone, 4-isopropyl thioxanthone, 2-chloro-thioxanthone, and 2, 4-diisopropyl thioxanthone;
the benzophenone photoinitiator is at least one selected from diphenyl ketone, 4-chlorine diphenyl ketone, methyl benzophenone, and 4-benzoyl-4'-methyl diphenyl thioether;
the acyl phosphine oxide photoinitiator is at least one selected from 2, 4, 6-trimethyl benzoyl diphenyl phosphine oxide, di-(2, 4, 6-trimethyl benzoyl)-phenyl phosphine oxide, di-(2, 6-dimethyl benzoyl)-2, 4, 4-trimethyl amyl phosphine oxide, and 2, 4, 6-trimethyl benzoyl phenyl ethyoxyl phosphine oxide;
the benzoate photoinitiator is methyl benzoylbenzoate, methyl ortho-benzoylbenzoate, or a mixture of them.

13. The method according to claim 7, wherein:
the curing process under infrared irradiation comprises: adjusting the infrared heating temperature to 20~150°C, allowing the release agent to flow flat for 0.01~10min., and curing the release agent;
the curing process under UV irradiation comprises: exposure to UV irradiation in an UV curing machine equipped with 1~3 ultraviolet lamps with 2-20Kw unit power and 0~3 metal halide lamps with 3~20Kw unit power, at 200-600nm wavelength, to cure the UV-curable protective paint, UV-curable ink, and UV-curable background paint, with the UV curing machine being operated at a conveying speed of 1~200m/min.

14. Use of the UV-curing transfer film according to any of claims 1 to 6 in the manufacture of an UV-curing transfer film decorative board.

15. The use according to claim 14, comprising:
applying a layer of UV-curable permeating agent on the surface of a fiber reinforced cement board, fiber reinforced calcium silicate board, fiber reinforced magnesium oxide board, light-weight magnesium chloride cement board, magnesium oxychloride board, or gypsum board, applying a layer of UV-curable paint filler on the surface of the UV-curable permeating agent, applying a layer of UV-curable sealing primer on the surface of the UV-curable paint filler, applying a layer of UV-curable pigmented paint on the surface of the UV-curable sealing primer, applying a layer of UV-curable glue on the surface of the UV-curable pigmented paint, and transferring the transfer film onto the UV-curable glue, to obtain the UV-curing transfer film decorative board; or
applying a layer of UV-curable sealing primer on the surface of a solid timber board, MDF board, or plywood board, applying a layer of UV-curable glue on the surface of the UV-curable sealing primer, and transferring the transfer film onto the surface of the UV-curable glue, to obtain the UV-curing transfer film decorative board; or
applying a layer of UV-curable metal primer on the surface of an aluminum plate, steel plate, or iron plate, applying a layer of UV-curable glue on the surface of the UV-curable metal primer, and transferring the transfer film onto the surface of the UV-curable glue, to obtain the UV-curing transfer film decorative plate.

## Patentansprüche

1. UV-härtende Transferfolie umfassend eine Substratfolie (10), eine Trennmittelschicht (2), eine UV-härtende Lackschutzschicht (3), eine UV-härtende dekorative Tintenmusterschicht (4) und eine UV-härtende Lackhintergrundschicht (5), wobei die Trennmittelschicht (2) sich auf der Substrattolie (1) befindet, die UV-härtende Lackschutzschicht (3) sich auf der Trennmittelschicht (2) befindet, die UV-härtende dekorative Tintenmusterschicht (4) sich auf der UV-härtenden Lackschutzschicht (3) befindet und die UV-härtende Lackhintergrundschicht (5) sich auf der UV-härtenden dekorativen Tintenmusterschicht (4) befindet,
wobei:
die Substrattolie (1) irgendeine ist von Polypropylenfolie, Polyethylenfolie, Polyvinylchloridfolie und Polyethylenterepththalattolie,
die Trennmittelschicht (2) durch ein Trennmittel gebildet ist, das eine Mischung von 20 - 50 Gew.-% Cellulose, 1 - 30 Gew.-% Wachs, 0 - 10 Gew.-% Siliconöl, 0 - 20 Gew.-% Butanon, 0~15 Gew.-% Ethylacetat, 5~20 Gew.-% Acrylatprepolymer, 5 - 20 Gew.-% Acrylatmonomer und 1 - 6 Gew.-% Photoinitiator ist,
die UV-härtende Lackschutzschicht (3) durch einen UV-härtbaren Lack gebildet ist, der eine Mischung von 10 ~ 80 Gew.-% Acrylatprepolymer, 5~50 Gew.-% Acrylatmonomer, 1 - 6 Gew.-% Photoinitiator, 0~2 Gew.-% Hilfsmittel, 0 ~ 50 Gew.-% Füllstoff, 0 - 10 Gew.-% Butanon und 0 - 15 Gew.-% Ethylacetat ist, oder
eine Mischung von 10 ~ 80 Gew.-% Acrylatprepolymer, 5 ~ 50 Gew.-% Acrylatmonomer, 1 - 6 Gew.-% Photoinitiator, 0 ~ 2 Gew.-% Hilfsmittel, 0 ~ 50 Gew.-% Füllstoff, 1 - 50 Gew.-% Mattiermittel, 0 - 10 Gew.-% Butanon und 0 ~ 15 Gew.-% Ethylacetat,
die UV-härtende dekorative Tintenmusterschicht (4) durch eine UV-härtbare Tinte gebildet ist, die eine Mischung von 10 ~ 60 Gew.-% Acrylatprepolymer, 5 ~ 50 Gew.-% Acrylatmonomer, 1 - 5 Gew.-% Photoinitiator, 0 ~ 2 Gew.-% Hilfsmittel, 0 - 50 Gew.-% Füllstoff, 5 ~ 30 Gew.-% Toner, 5 ~ 30 Gew.-% Harz, 0 ~ 10 Gew.-% Butanon und 0 - 15 Gew.-% Ethylacetat ist, und
die UV-härtende Lackhintergrundschicht (5) durch einen UV-härtbaren Lack gebildet ist, der eine Mischung von 10 ~ 50 Gew.-% Acrylatprepolymer, 10 ~ 40 Gew.-% Acrylatmonomer, 1 - 5 Gew.-% Photoinitiator, 0 ~ 2 Gew.-% Hilfsmittel, 0 -30 Gew.-% Füllstoff, 5 ~ 30 Gew.-% Toner, 5 ~ 50 Gew.-% Harz, 0 ~ 10 Gew.-% Butanon und 0 ~ 15 Gew.-% Ethylacetat ist.

2. UV-härtende Transferfolie nach Anspruch 1, wobei:
die Cellulose Methylolcellulose ist,
das Wachs modifiziertes Paraffinwachs, Palmwachs, eine Mischung davon ist,
das Siliconöl mindestens eines ist ausgewählt von Methylsiliconöl, Benzilsiliconöl und Hydroxysiliconol.

3. UV-härtende Transferfolie nach Anspruch 1 oder 2, wobei: die Polypropylenfolie eine modifizierte Polypropylenfolie ist.

4. UV-härtende Transferfolie nach einem der Ansprüche 1 bis 3, wobei:
das Acrylatprepolymer mindestens eines ist ausgewählt von Epoxyacrylat, fluorhaltigem Epoxyacrylat, Polyurethanacrylat, fluorhaltigem Polyurethanacrylat, Polyesteracrylat, fluorhaltigem Polyesteracrylat, Aminoacrylat, fluorhaltigem Aminoacrylat, Acrylatcopolymer und fluorhaltigem Acrylatcopolymer,
das Acrylatmonomer mindestens eines ist ausgewählt von Butylacrylat, Cyclohexylacrylat, Ethylhexylacrylat, Hydroxyethylacrylat, Hydroxyethylmethacrylat, Trifluorethylacrylat, Trifluorethylmethacrylat, Hexafluorbutylacrylat, Hexafluorbutylmethacrylat, Dodecafluorheptylacrylat, Dodecafluorheptylmethacrylat, Tripropylenglycoldiacrylat, Dipropylenglycoldiacrylat, Neopentylglycoldiacrylat, Propoxyneopentylglycoldiacrylat, Phthalandion-di-(diethylenglycol)diacrylat, 1,6-Hexylenglycoldiacrylat, Trimethylolpropantriacrylat, Ethoxytrimethylolpropantriacrylat, Propoxytrimethylolpropantriacrylat, Pentaerythrittriacrylat und Dipentaerythrithexaacrylat,
der Photoinitiator mindestens einer ist ausgewählt von Benzoinetherphotoinitiator, Benzilketalphotoinitiator, Acetophenonphotoinitiator, Anthrachinonphotoinitiator, Thioxanthonphotoinitiator, Benzophenonphotoinitiator, Acylphosphinoxidphotoinitiator und Benzoatphotoinitiator,
das Harz mindestens eines ist ausgewählt von modifiziertem Polyvinylacetat, Polyamidharz und thermoplastischem Acryl,
der Toner mindestens einer ist ausgewählt von Rußkohlenstoff, Titanpigment, Phthalocyanin-blau, Proflavin und Scharlachrotpulver,
das Hilfsmittel mindestens eines ist ausgewählt von Egalisiermittel, Antischaummittel und Benetzungsmittel und Dispergiermittel,
der Füllstoff mindestens eines ist ausgewählt von Talkumpuder, Calciumcarbonat und Bariumsulfat,
das Mattiermittel Mattierwachs, Mattierpulver oder eine Mischung davon ist.

5. UV-härtende Transferfolie nach Anspruch 4, wobei das modifizierte Polyvinylacetat Vinylchloridvinylacetat, Ethylenvinylacetat oder eine Mischung davon ist.

6. UV-härtende Transferfolie nach Anspruch 4, wobei:
der Benzoinetherphotoinitiator mindestens einer ist ausgewählt von Benzoinmethylether, Benzoinethylether und Benzoinisopropylether,
der Benzilketalphotoinitiator Benzildimethylketal ist,
der Acetophenonphotoinitiator mindestens einer ist ausgewählt von Acetophenon, 2,2-Dimethoxy-2-phenylacetophenon, 2,2-Diethoxy-2-phenylacetophenon, 1,1-Dichloracetophenon, 1-Hydroxylacetophenon, 1-Hydroxylcyclohexylphenylketon, 2-Hydroxyl-2-methyl-1-phenyl-1-aceton, 1-(4-Isopropylphenyl)-2-hydroxyl-2-methyl-1-aceton, 1-[4-(2-Hydroxylethoxyl)phenyl]-2-hydroxyl-2-methyl-1-aceton, 2-Methyl-1-[4-(methylsulfenyl)phenyl]-2-morpholinyl-1-aceton und 1-Benzyl-2-dimethylamido-1 (4-morpholinylphenyl)-1-butanon,
der Anthrachinonphotoinitiator mindestens einer ist ausgewählt von 2-tert.-Butylanthrachinon, 1-Chloranthrachinon, und 2-Amylanthrachinon,
der Thioxanthonphotoinitiator mindestens einer ist ausgewählt von 2,4-Dimethylthioxanthon, 2,4-Diethylthioxanthon, 2-Isopropylthioxanthon, 4-Isopropylthioxanthon, 2-Chlorthioxanthon und 2,4-Diisopropylthioxanthon,
der Benzophenonphotoinitiator mindestens einer ist ausgewählt von Diphenylketon, 4-Chlordiphenylketon, Methylbenzophenon und 4-Benzoyl-4'-methyldiphenyltthioether,
der Acylphosphinoxidphotoinitiator mindestens einer ist ausgewählt von 2,4,6-Trimethylbenzoyldiphenylphosphinoxid, Di-(2,4,6-Trimethylbenzoyl)phenylphosphinoxid, Di-(2,6-dimethylbenzoyl)-2,4,4-trimethylamylphosphinoxid und 2,4,6-Trimethylbenzoylphenylethoxylphosphinoxid,
der Benzoatphotoinitiator Methylbenzoylbenzoat, Methylorthobenzoylbenzoat oder eine Mischung davon ist.

7. Verfahren für die Herstellung der UV-härtende Transferfolie nach einem der Ansprüche 1 bis 6, einschließlich des: gleichförmig schichtförmigen Aufbringens oder Druckens eines Trennmittels auf eine Substratfolie (1) und dann Härtens des Trennmittels durch Infrarotstrahlung, um eine Trennmittelschicht (2) auf der Substratfolie (1) zu erhalten; gleichförmig schichtförmigen Aufbringens oder Druckes von UV-härtbarem Schutzlack auf die Trennmittelschicht (2) und dann Härtens des Lacks durch UV-Strahlung, um eine UV-härtende Lackschutzschicht (3) zu erhalten; gleichförmig schichtförmigen Aufbringens oder Druckes von UV-härtbarer Tinte, die Muster und eine dekorative Wirkung auf der UV-härtenden Lackschutzschicht (3) aufweist, und dann Härtens der Tinte durch UV-Strahlung, um eine UV-härtende dekorative Tintenmusterschicht (4) zu erhalten; und gleichförmig schichtförmigen Aufbringens oder Druckes von UV-härtbarem Hintergrundlack auf die UV-härtende dekorative Tintenmusterschicht (4) und dann Härtens des Lacks durch UV-Strahlung, um eine UV-härtende Transferfolie zu erhalten, wobei:
die Substratfolie (1) irgendeine von Polypropylenfolie, Polyethylenfolie, Polyvinylchloridfolie und Polyethylenterepththalatfolie ist,
die Trennmittelschicht (2) durch ein Trennmittel gebildet ist, das eine Mischung ist von 20 - 50 Gew.-% Cellulose, 1 - 30 Gew.-% Wachs, 0 - 10 Gew.-% Siliconöl, 0 - 20 Gew.-% Butanon, 0 ~ 15 Gew.-% Ethylacetat, 5 ~ 20 Gew.-% Acrylatprepolymer, 5 - 20 Gew.-% Acrylatmonomer und 1 ~ 6 Gew.-% Photoinitiator,
die UV-härtende Lackschutzschicht (3) durch einen UV-härtbaren Lack gebildet ist, der eine Mischung von 10 ~ 80 Gew.-% Acrylatprepolymer, 5 ~ 50 Gew.-% Acrylatmonomer, 1 - 6 Gew.-% Photoinitiator, 0 ~ 2 Gew.-% Hilfsmittel, 0 ~ 50 Gew.-% Füllstoff, 0 ~ 10 Gew.-% Butanon und 0 ~ 15 Gew.-% Etyhlacetat ist; oder eine Mischung von 10 ~ 80 Gew.-% Acrylatprepolymer, 5 ~ 50 Gew.-% Acrylatmonomer, 1 - 6 Gew.-% Photoinitiator, 0 ~ 2 Gew.-% Hilfsmittel, 0 ~ 50 Gew.-% Füllstoff, 1 ~ 50 Gew.-% Mattiermittel, 0 ~ 10 Gew.-% Butanon und 0 ~ 15 Gew.-% Ethylacetat,
die UV-härtende dekorative Tintenmusterschicht (4) durch eine UV-härtbare Tinte gebildet ist, die eine Mischung von 10 ~ 60 Gew.-% Acrylatprepolymer, 5 ~ 50 Gew.-% Acrylatmonomer, 1 - 5 Gew.-% Photoinitiator, 0 ~ 2 Gew.-% Hilfsmittel, 0 - 50 Gew.-% Füllstoff, 5 ~ 30 Gew.-% Toner, 5 ~ 30 Gew.-% Harz, 0 ~ 10 Gew.-% Butanon und 0 ~ 15 Gew.-% Ethylacetat,
die UV-härtende Lackhintergrundschicht (5) durch einen UV-härtenden Lack gebildet ist, der eine Mischung von 10 ~ 50 Gew.-% Acrylatprepolymer, 10 ~ 40 Gew.-% Acrylatmonomer, 1 - 5 Gew.-% Photoinitiator, 0 ~ 2 Gew.-% Hilfsmittel, 0 -30 Gew.-% Füllstoff, 5 ~ 30 Gew.-% Toner, 5 ~ 50 Gew.-% Harz, 0 - 10 Gew.-% Butanon und 0 ~ 15 Gew.-% Ethylacetat ist.

8. Verfahren nach Anspruch 7, wobei:
die Cellulose Methylolcellulose ist,
das Wachs modifiziertes Paraffinwachs, Palmwachs, eine Mischung davon ist,
das Siliconöl mindestens eines ist ausgewählt von Methylsiliconöl, Benzilsiliconöl und Hydroxysiliconol.

9. Verfahren nach den Ansprüchen 7 oder 8, wobei: die Polypropylenfolie eine modifizierte Polypropylenfolie ist.

10. Verfahren nach einem der Ansprüche 7 bis 9, wobei:
das Acrylatprepolymer mindestens eines ist ausgewählt von Epoxyacrylat, fluorhaltigem Epoxyacrylat, Polyurethanacrylat, fluorhaltigem Polyurethanacrylat, Polyesteracrylat, fluorhaltigem Polyesteracrylat, Aminoacrylat, fluorhaltigem Aminoacrylat, Acrylatcopolymer und fluorhaltigem Acrylatcopolymer,
das Acrylatmonomer mindestens eines ist ausgewählt von Butylacrylat, Cyclohexylacrylat, Ethylhexylacrylat, Hydroxyethylacrylat, Hydroxyethylmethacrylat, Trifluorethylacrylat, Trifluorethylmethacrylat, Hexafluorbutylacrylat, Hexafluorbutylmethacrylat, Dodecafluorheptylacrylat, Dodecafluorheptylmethacrylat, Tripropylenglycoldiacrylat, Dipropylenglycoldiacrylat, Neopentylglycoldiacrylat, Propoxyneopentylglycoldiacrylat, Phthalandion-di-(diethylenglycol)diacrylat, 1,6-Hexylenglycoldiacrylat, Trimethylolpropantriacrylat, Ethoxytrimethylolpropantriacrylat, Propoxytrimethylolpropantriacrylat, Pentaerythrittriacrylat und Dipentaerythrithexaacrylat,
der Photoinitiator mindestens einer ist ausgewählt von Benzoinetherphotoinitiator, Benzilketalphotoinitiator, Acetophenonphotoinitiator, Anthrachinonphotoinitiator, Thioxanthonphotoinitiator, Benzophenonphotoinitiator, Acylphosphinoxidphotoinitiator und Benzoatphotoinitiator,
das Harz mindestens eines ist ausgewählt von modifiziertem Polyvinylacetat, Polyamid harz und thermoplastischem Acryl,
der Toner mindestens einer ist ausgewählt von Rußkohlenstoff, Titanpigment, Phthalocyanin-blau, Proflavin und Scharlachrotpulver,
das Hilfsmittel mindestens eines ist ausgewählt von Egalisiermittel, Antischaummittel und Benetzungsmittel und Dispergiermittel,
der Füllstoff mindestens eines ist ausgewählt von Talkumpuder, Calciumbentonat und Bariumsulfat; das Mattiermittel ein Mattierwachs, Mattierpulver oder eine Mischung davon ist.

11. Verfahren nach Anspruch 10, wobei: das modifizierte Polyvinylacetat Vinylchloridvinylacetat, Ethylenvinylacetat oder eine Mischung davon ist.

12. Verfahren nach einem der Ansprüche 10 bis 11, wobei: der Benzoinetherphotoinitiator mindestens einer ist ausgewählt von Benzoinmethylether, Benzoinethylether und Benzoinisopropylether,
der Benzilketalphotoinitiator Benzildimethylketal ist,
der Acetophenonphotoinitiator mindestens einer ist ausgewählt von Acetophenon, 2,2-Dimethoxy-2-phenylacetophenon, 2,2-Diethoxy-2-phenylacetophenon, 1,1-Dichloracetophenon, 1-Hydroxylacetophenon, 1-Hydroxylcyclohexylphenylketon, 2-Hydroxyl-2-methyl-1-phenyl-1-aceton, 1-(4-Isopropylphenyl)-2-hydroxyl-2-methyl-1-aceton, 1-[4-(2-Hydroxylethoxyl)phenyl]-2-hydroxyl-2-methyl-1-aceton, 2-Methyl-1-[4-(methylsulfenyl)phenyl]-2-morpholinyl-1-aceton und 2-Benzyl-2-dimethylamido-1 (4-morpholinylphenyl)-1-butanon,
der Anthrachinonphotoinitiator mindestens einer ist ausgewählt von 2-tert.-Butylanthrachinon, 1-Chloranthrachinon und 2-Amylanthrachinon,
der Thioxanthonphotoinitiator mindestens einer ist ausgewählt von 2,4-Dimethylthioxanthon, 2,4-Diethylthioxanthon, 2-Isopropylthioxanthon, 4-Isopropylthioxanthon, 2-Chlorthioxanthon und 2,4-Diisopropylthioxanthon,
der Benzophenonphotoinitiator mindestens einer ist ausgewählt von Diphenylketon, 4-Chlordiphenylketon, Methylbenzophenon und 4-Benzoyl-4'-methyldiphenyltthioether,
der Acylphosphinoxidphotoinitiator mindestens einer ist ausgewählt von 2,4,6-Trimethylbenzoyldiphenylphosphinoxid, Di-(2,4,6-Trimethylbenzoyl)phenylphosphinoxid, Di-(2,6-dimethylbenzoyl)-2,4,4-thrimethylamylphosphinoxid und 2,4,6-Trimethylbenzoylphenylethoxylphosphinoxid,
der Benzoatphotoinitiator Methylbenzoylbenzoat, Methylorthobenzoylbenzoat oder eine Mischung davon ist.

13. Verfahren nach Anspruch 7, wobei:
der Härtungsvorgang unter Infrarotstrahlung Folgendes umfasst: das Einstellen der Infraroterhitzungstemperatur auf 20 ~ 150 °C, was es dem Trennmittel gestattet, 0,01~10 min lang zu fließen, und Härten des Trennmittels,
der Härtungsvorgang unter UV-Strahlung Folgendes umfasst: Aussetzen an UV-Strahlung in einer UV-Härtungsmaschine, die mit 1 - 3 Ultraviolettlampen mit einer Einheitsleistung von 2 ~ 20 kW und 0 ~ 3 Metallhalogenidlampen mit einer Einheitsleistung von 3 ~ 20 kW ausgestattet ist, bei einer Wellenlänge von 200 ~ 600 nm, um den UV-härtbaren Schutzlack, die UV-härtbare Tinte und den UV-härtbaren Hintergrundlack zu härten, wobei die UV-Härtungsmaschine mit einer Fördergeschwindigkeit von 1 - 200 m/min betrieben wird.

14. Verwendung der UV-härtbaren Transferfolie nach einem der Ansprüche 1 bis 6 bei der Fertigung einer UV-härtenden dekorativen Transferfolienplatte.

15. Verwendung nach Anspruch 14, umfassend:
das Aufbringen einer Schicht UV-härtbaren Durchdringungsmitteln auf die Oberfläche einer faserverstärkten Zementplatte, faserverstärkten Calciumsilicatplatte, faserverstärkten Magnesiumoxidplatte, Magnesiumchloridzementplatte von leichtem Gewicht, Magnesiumoxychloridplatte oder Gipsplatte, das Aufbringen einer Schicht UV-härtbaren Lackfüllstoffs auf die Oberfläche des UV-härtbaren Durchdringungsmittels, das Aufbringen einer Schicht UV-härtbaren Abdichtgrundiermittels auf die Oberfläche des UV-härtbaren Lackfüllstoffs, das Aufbringen einer Schicht UV-härtbaren pigmentierten Lacks auf die Oberfläche des UV-härtbaren Abdichtgrundiermittels, das Aufbringen einer Schicht UV-härtbaren Klebstoffs auf die Oberfläche des UV-härtbaren pigmentierten Lacks und das Übertragen der Transferfolie auf den UV-härtbaren Klebstoff, um eine UV-härtende dekorative Transferfolienplatte zu erhalten, oder
das Aufbringen einer Schicht UV-härtbarem Abdichtgrundiermittels auf die Oberfläche einer Massivholzplatte, mitteldichten Holzfaserplatte oder Sperrholzplatte, das Aufbringen einer Schicht UV-härtbaren Klebstoffs auf die Oberfläche des UV-härtbaren Abdichtgrundiermittels und das Übertragen der Transferfolie auf die Oberfläche des UV-härtbaren Klebstoffs, um die UV-härtende dekorative Transferfolienplatte zu erhalten, oder
das Aufbringen einer Schicht UV-härtbaren Metallgrundiermittels auf die Oberfläche einer Aluminiumplatte, Stahlplatte oder Eisenplatte, das Aufbringen einer Schicht UV-härtbaren Klebstoffs auf die Oberfläche des UV-härtbaren Metallgrundiermittels und das Übertragen der Transferfolie auf die Oberfläche des UV-härtbaren Klebstoffs, um die UV-härtende dekorative Transferfolienplatte zu erhalten.

## Revendications

1. Film de transfert durcissable aux UV, comprenant un film de substrat (1), une couche d'agent de séparation (2), une couche protectrice de peinture durcissable aux UV (3), une couche de motif décoratif d'encre durcissable aux UV (4), et une couche de fond de peinture durcissable aux UV (5), la couche d'agent de séparation (2) étant sur le film de substrat (1), la couche protectrice de peinture durcissable aux UV (3) étant sur la couche d'agent de séparation (2), la couche de motif décoratif d'encre durcissable aux UV (4) étant sur la couche protectrice de peinture durcissable aux UV (3), et la couche de fond de peinture durcissable aux UV (5) est sur la couche de motif décoratif d'encre durcissable aux UV (4) ;
dans lequel :
le film de substrat (1) est l'un quelconque d'un film de polypropylène, un film de polyéthylène, un film de chlorure de polyvinyle, et un film de polyéthylène-téréphtalate ;
la couche d'agent de séparation (2) est formée d'un agent de séparation qui est un mélange de 20 à 50 % en poids de cellulose, 1 à 30 % en poids de cire, 0 à 10 % en poids d'huile de silicone, 0 à 20 % en poids de butanone, 0 à 15 % en poids d'acétate d'éthyle, 5 à 20 % en poids de prépolymère d'acrylate, 5 à 20 % en poids de monomère d'acrylate, et 1 à 6 % en poids de photo-initiateur ;
la couche protectrice de peinture durcissable aux UV (3) est formée d'une peinture durcissable aux UV qui est un mélange de 10 à 80 % en poids de prépolymère d'acrylate, 5 à 50 % en poids de monomère d'acrylate, 1 à 6 % en poids de photo-initiateur, 0 à 2 % en poids d'agent auxiliaire, 0 à 50 % en poids de charge, 0 à 10 % en poids de butanone, et 0 à 15 % en poids d'acétate d'éthyle ; ou
un mélange de 10 à 80 % en poids de prépolymère d'acrylate, 5 à 50 % en poids de monomère d'acrylate, 1 à 6 % en poids de photo-initiateur, 0 à 2 % en poids d'agent auxiliaire, 0 à 50 % en poids de charge, 1 à 50 % en poids d'agent de matage, 0 à 10 % en poids de butanone, et 0-15 % en poids d'acétate d'éthyle ;
la couche de motif décoratif d'encre durcissable aux UV (4) est formée d'une encre durcissable aux UV qui est un mélange de 10 à 60 % en poids de prépolymère d'acrylate, 5 à 50 % en poids de monomère d'acrylate, 1 à 5 % en poids de photoinitiateur, 0 à 2 % en poids d'agent auxiliaire, 0 à 50 % en poids de charge, 5 à 30 % en poids de toner, 5 à 30 % en poids de résine, 0 à 10 % en poids de butanone, et 0 à 15 % en poids d'acétate d'éthyle ; et
la couche de fond de peinture durcissable aux UV (5) est formée d'une peinture durcissable aux UV qui est un mélange de 10 à 50 % en poids de prépolymère d'acrylate, 10 à 40 % en poids de monomère d'acrylate, 1 à 5 % en poids de photoinitiateur, 0 à 2 % en poids d'agent auxiliaire, 0 à 30 % en poids de charge, 5 à 30 % en poids de toner, 5 à 50 % en poids de résine, 0 à 10 % en poids de butanone, et 0 à 15 % en poids d'acétate d'éthyle.

2. Film de transfert durcissable aux UV selon la revendication 1, dans lequel :
la cellulose est de la méthylolcellulose ;
la cire est de la cire de paraffine modifiée, de la cire de palme, ou un mélange de celles-ci ;
l'huile de silicone est au moins l'une choisie parmi l'huile de méthylsilicone, l'huile de benzylsilicone, et l'huile d'hydroxylsilicone.

3. Film de transfert durcissable aux UV selon la revendication 1 ou 2, dans lequel le film de polypropylène est un film de polypropylène modifié.

4. Film de transfert durcissable aux UV selon l'une quelconque des revendications 1 à 3, dans lequel :
le prépolymère d'acrylate est au moins l'un choisi parmi époxy acrylate, époxy acrylate contenant du fluor, polyuréthane acrylate, polyuréthane acrylate contenant du fluor, polyester acrylate, polyester acrylate contenant du fluor, amino acrylate, amino acrylate contenant du fluor, un copolymère d'acrylate, et un copolymère d'acrylate contenant du fluor ;
le monomère d'acrylate est au moins l'un choisi parmi l'acrylate de butyle, l'acrylate de cyclohexyle, l'acrylate d'éthylhexyle, l'acrylate d'hydroxyéthyle, le méthacrylate d'hydroxyéthyle, l'acrylate de trifluoroéthyle, le méthacrylate de trifluoroéthyle, l'acrylate d'hexafluorobutyle, le méthacrylate d'hexafluorobutyle, l'acrylate de dodécafluoroheptyle, le méthacrylate de dodécafluoroheptyle, le diacrylate de tripropylène glycol, le diacrylate de dipropylène glycol, le diacrylate de néopentylglycol, le diacrylate de propoxy-néopentylglycol, le diacrylate de phtalandione di-(diéthylèneglycol), le diacrylate de 1,6-hexylène glycol, le triacrylate de triméthylolpropane, le triacrylate d'éthoxy-triméthylolpropane, le triacrylate de propoxy-triméthylolpropane, le triacrylate de pentaérythritol, et l'hexa-acrylate de dipentaérythritol ;
le photo-initiateur est au moins l'un choisi parmi un photo-initiateur d'éther de benzoïne, un photo-initiateur de benzil-kétal, un photo-initiateur d'acétophénone, un photo-initiateur d'anthraquinone, un photo-initiateur de thioxanthone, un photo-initiateur de benzophénone, un photo-initiateur d'oxyde d'acyl-phosphine, et un photo-initiateur de benzoate,
la résine est au moins l'une choisi parmi le polyacétate de vinyle modifié, une résine polyamide, et un acrylique thermoplastique ;
le toner est au moins l'un choisi parmi du carbone de suie, un pigment au titane, le bleu de phtalocyanine, la proflavine, et de la poudre écarlate,
l'agent auxiliaire est au moins l'un choisi parmi un agent révélant, un agent antimousse, et un agent mouillant et dispersant ;
la charge est au moins l'un choisi parmi la poudre de talc, le carbonate de calcium, et le sulfate de baryum ;
l'agent de matage est une cire de matage, une poudre de matage, ou un mélange de celles-ci.

5. Film de transfert durcissable aux UV selon la revendication 4, dans lequel : le polyacétate de vinyle modifié est du chlorure de vinyle-acétate de vinyle, de l'éthylène-acétate de vinyle, ou un mélange de ceux-ci.

6. Film de transfert durcissable aux UV selon la revendication 4, dans lequel :
le photo-initiateur d'éther de benzoïne est au moins l'un choisi parmi l'éther méthylique de benzoïne, l'éther éthylique de benzoïne, et l'éther isopropylique de benzoïne ;
le photo-initiateur de benzil-kétal est le benzil-diméthyl-kétal ;
le photo-initiateur d'acétophénone est au moins l'un choisi parmi l'acétophénone, la 2,2-di-méthoxy-2-phényl-acétophénone, la 2,2-diéthoxy-2-phényl-acétophénone, la 1,1-dichloro-acétophénone, la 1-hydroxyl-acétophénone, la 1-hydroxyl-cyclohexyl-phénylcétone, la 2-hydroxyl-2-méthyl-1-phényl-1-acétone, la 1-(4-isopropylphényl)-2-hydroxyl-2-méthyl-acétone, la 1-[4-(2-hydroxyléthyoxyl)phényl]-2-hydroxyl-2-méthyl-1-acétone, la 2-méthyl-1-[4-(méthylsulfényl)phényl]-2-morpholinyl-1-acétone, et la 2-benzyl-2-diméthylamido-1-(4-morpholinylphényl)-1-butanone ;
le photo-initiateur d'anthraquinone est au moins l'un choisi parmi la 2-tert-butyl-anthraquinone, la 1-chloro-anthraquinone, et la 2-amyl-anthraquinone ;
le photo-initiateur de thioxanthone est au moins l'un choisi parmi la 2,4-diméthyl-thioxanthone, la 2,4-diéthyl-thioxanthone, la 2-isopropyl-thioxanthone, la 4-isopropyl-thioxanthone, la 2-chloro-thioxanthone, et la 2,4-düsopropyl-thioxanthone ; le photo-initiateur de benzophénone est au moins l'un choisi parmi la diphénylcétone, la 4-chlorodiphénylcétone, la méthyl-benzophénone, et le thioéther 4-benzoyl-4'-méthyl-diphénylique ;
le photo-initiateur d'oxyde d'acyl-phosphine est au moins l'un choisi parmi l'oxyde de 2,4,6-triméthyl-benzoyl-diphényl-phosphine, l'oxyde de di-(2,4,6-triméthyl-benzoyl)-phényl-phosphine, l'oxyde de di-(2,6-diméthyl-benzoyl)-2,4,4-triméthylamyl-phosphine, et l'oxyde de 2,4,6-triméthylbenzoylphényléthyoxyl-phosphine ;
le photo-initiateur de benzoate est le benzoylbenzoate de méthyle, l'ortho-benzoylbenzoate de méthyle, ou un mélange de ceux-ci.

7. Procédé pour la préparation du film de transfert durcissable aux UV selon l'une quelconque des revendications 1 à 6, comprenant : l'enduction ou l'impression uniformes d'un agent de séparation sur un film de substrat (1), et ensuite le durcissement de l'agent de séparation par irradiation infrarouge, pour obtenir une couche d'agent de séparation (2) sur le film de substrat (1) ; l'enduction ou l'impression uniformes de peinture protectrice durcissable aux UV sur la couche d'agent de séparation (2), et ensuite le durcissement de la peinture par irradiation UV, pour obtenir une couche protectrice de peinture durcissable aux UV (3) ; l'enduction ou l'impression uniformes d'une encre durcissable aux UV qui a des motifs et un effet décoratif sur la couche protectrice de peinture durcissable aux UV (3), et ensuite le durcissement de l'encre par irradiation UV, pour obtenir une couche de motif décoratif d'encre durcissable aux UV (4) ; et l'enduction ou l'impression uniformes de peinture de fond durcissable aux UV sur la couche de motif décoratif d'encre durcissable aux UV (4), et ensuite le durcissement de la peinture par irradiation UV, pour obtenir le film de transfert durcissable aux UV, où :
le film de substrat (1) est l'un quelconque d'un film de polypropylène, un film de polyéthylène, un film de chlorure de polyvinyle, et un film de polyéthylène-téréphtalate ;
la couche d'agent de séparation (2) est formée d'un agent de séparation qui est un mélange de 20 à 50 % en poids de cellulose, 1 à 30 % en poids de cire, 0 à 10 % en poids d'huile de silicone, 0 à 20 % en poids de butanone, 0 à 15 % en poids d'acétate d'éthyle, 5 à 20 % en poids de prépolymère d'acrylate, 5 à 20 % en poids de monomère d'acrylate, et 1 à 6 % en poids de photo-initiateur ;
la couche protectrice de peinture durcissable aux UV (3) est formée d'une peinture durcissable aux UV qui est un mélange de 10 à 80 % en poids de prépolymère d'acrylate, 5 à 50 % en poids de monomère d'acrylate, 1 à 6 % en poids de photoinitiateur, 0 à 2 % en poids d'agent auxiliaire, 0 à 50 % en poids de charge, 0 à 10 % en poids de butanone, et 0 à 15 % en poids d'acétate d'éthyle ; ou un mélange de 10 à 80 % en poids de prépolymère d'acrylate, 5 à 50 % en poids de monomère d'acrylate, 1 à 6 % en poids de photo-initiateur, 0 à 2 % en poids d'agent auxiliaire, 0 à 50 % en poids de charge, 1 à 50 % en poids d'agent de matage, 0 à 10 % en poids de butanone, et 0 à 15 % en poids d'acétate d'éthyle ;
la couche de motif décoratif d'encre durcissable aux UV (4) est formée d'une encre durcissable aux UV qui est un mélange de 10 à 60 % en poids de prépolymère d'acrylate, 5 à 50 % en poids de monomère d'acrylate, 1 à 5 % en poids de photo-initiateur, 0 à 2 % en poids d'agent auxiliaire, 0 à 50 % en poids de charge, 5 à 30 % en poids de toner, 5 à 30 % en poids de résine, 0 à 10 % en poids de butanone, et 0 à 15 % en poids d'acétate d'éthyle ;
la couche de fond de peinture durcissable aux UV (5) est formée d'une peinture durcissable aux UV qui est un mélange de 10 à 50 % en poids de prépolymère d'acrylate, 10 à 40 % en poids de monomère d'acrylate, 1 à 5 % en poids de photo-initiateur, 0 à 2 % en poids d'agent auxiliaire, 0 à 30 % en poids de charge, 5 à 30 % en poids de toner, 5 à 50 % en poids de résine, 0 à 10 % en poids de butanone, et 0 à 15 % en poids d'acétate d'éthyle.

8. Procédé selon la revendication 7, dans lequel :
la cellulose est la méthylolcellulose ;
la cire est de la cire de paraffine modifiée, de la cire de palme, ou un mélange de celles-ci ;
l'huile de silicone est au moins l'une choisie parmi l'huile de méthylsilicone, l'huile de benzylsilicone, et l'huile d'hydroxylsilicone.

9. Procédé selon les revendications 7 ou 8, dans lequel : le film de polypropylène est un film de polypropylène modifié.

10. Procédé selon l'une quelconque des revendications 7 à 9, dans lequel :
le prépolymère d'acrylate est au moins l'un choisi parmi époxy acrylate, époxy acrylate contenant du fluor, polyuréthane acrylate, polyuréthane acrylate contenant du fluor, polyester acrylate, polyester acrylate contenant du fluor, amino acrylate, amino acrylate contenant du fluor, un copolymère d'acrylate, et un copolymère d'acrylate contenant du fluor ;
le monomère d'acrylate est au moins l'un choisi parmi l'acrylate de butyle, l'acrylate de cyclohexyle, l'acrylate d'éthylhexyle, l'acrylate d'hydroxyéthyle, le méthacrylate d'hydroxyéthyle, l'acrylate de trifluoroéthyle, le méthacrylate de trifluoroéthyle, l'acrylate d'hexafluorobutyle, le méthacrylate d'hexafluorobutyle, l'acrylate de dodécafluoroheptyle, le méthacrylate de dodécafluoroheptyle, le diacrylate de tripropylène glycol, le diacrylate de dipropylène glycol, le diacrylate de néopentylglycol, le diacrylate de propoxy-néopentylglycol, le diacrylate de phtalandione di-(diéthylèneglycol), le diacrylate de 1,6-hexylène glycol, le triacrylate de triméthylolpropane, le triacrylate d'éthoxy-triméthylolpropane, le triacrylate de propoxy-triméthylolpropane, le triacrylate de pentaérythritol, et l'hexa-acrylate de dipentaérythritol ;
le photo-initiateur est au moins l'un choisi parmi un photo-initiateur d'éther de benzoïne, un photo-initiateur de benzil-kétal, un photo-initiateur d'acétophénone, un photo-initiateur d'anthraquinone, un photo-initiateur de thioxanthone, un photo-initiateur de benzophénone, un photo-initiateur d'oxyde d'acyl-phosphine, et un photo-initiateur de benzoate,
la résine est au moins l'une choisi parmi le polyacétate de vinyle modifié, une résine polyamide, et un acrylique thermoplastique ;
le toner est au moins l'un choisi parmi du carbone de suie, un pigment au titane, le bleu de phtalocyanine, la proflavine, et de la poudre écarlate,
l'agent auxiliaire est au moins l'un choisi parmi un agent révélant, un agent antimousse, et un agent mouillant et dispersant ;
la charge est au moins l'un choisi parmi la poudre de talc, le carbonate de calcium, et le sulfate de baryum ; l'agent de matage est une cire de matage, une poudre de matage, ou un mélange de celles-ci.

11. Procédé selon la revendication 10, dans lequel : le polyacétate de vinyle modifié est chlorure de vinyle-acétate de vinyle, éthylène-acétate de vinyle, ou un mélange de ceux-ci.

12. Procédé selon l'une quelconque des revendications 10 à 11, dans lequel :
le photo-initiateur d'éther de benzoïne est au moins l'un choisi parmi l'éther méthylique de benzoïne, l'éther éthylique de benzoïne, et l'éther isopropylique de benzoïne ;
le photo-initiateur de benzil-kétal est le benzil-diméthyl-kétal ;
le photo-initiateur d'acétophénone est au moins l'un choisi parmi l'acétophénone, la 2,2-di-méthoxy-2-phényl-acétophénone, la 2,2-diéthoxy-2-phényl-acétophénone, la 1,1-dichloro-acétophénone, la 1-hydroxyl-acétophénone, la 1-hydroxyl-cyclohexyl-phénylcétone, la 2-hydroxyl-2-méthyl-1-phényl-1-acétone, la 1-(4-isopropylphényl)-2-hydroxyl-2-méthyl-acétone, la 1-[4-(2-hydroxyléthyoxyl)phényl]-2-hydroxyl-2-méthyl-1-acétone, la 2-méthyl-1-[4-(méthylsulfényl)phényl]-2-morpholinyl-1-acétone, et la 2-benzyl-2-diméthylamido-1-(4-morpholinylphényl)-1-butanone ;
le photo-initiateur d'anthraquinone est au moins l'un choisi parmi la 2-tert-butyl-anthraquinone, la 1-chloro-anthraquinone, et la 2-amyl-anthraquinone ;
le photo-initiateur de thioxanthone est au moins l'un choisi parmi la 2,4-diméthyl-thioxanthone, la 2,4-diéthyl-thioxanthone, la 2-isopropyl-thioxanthone, la 4-isopropyl-thioxanthone, la 2-chloro-thioxanthone, et la 2,4-düsopropyl-thioxanthone ;
le photo-initiateur de benzophénone est au moins l'un choisi parmi la diphénylcétone, la 4-chlorodiphénylcétone, la méthyl-benzophénone, et le thioéther 4-benzoyl-4'-méthyl-diphénylique ;
le photo-initiateur d'oxyde d'acyl-phosphine est au moins l'un choisi parmi l'oxyde de 2,4,6-triméthyl-benzoyl-diphényl-phosphine, l'oxyde de di-(2,4,6-triméthyl-benzoyl)-phényl-phosphine, l'oxyde de di-(2,6-diméthyl-benzoyl)-2,4,4-triméthylamyl-phosphine, et l'oxyde de 2,4,6-triméthylbenzoylphényléthyoxyl-phosphine ;
le photo-initiateur de benzoate est le benzoylbenzoate de méthyle, l'ortho-benzoylbenzoate de méthyle, ou un mélange de ceux-ci.

13. Procédé selon la revendication 7, dans lequel :
le procédé de durcissement sous irradiation infrarouge comprend : l'ajustement de la température de chauffage infrarouge à 20 à 150 °C, l'étape consistant à laisser l'agent de séparation s'écouler à plat pendant 0,01 à 10 min., et le durcissement de l'agent de séparation ;
le procédé de durcissement sous irradiation UV comprend : l'exposition à une irradiation UV dans une machine de durcissement UV équipée d'une à trois lampes ultraviolettes ayant une puissance unitaire de 2 à 20 Kw est zéro à trois lampes à halogénures de métal ayant une puissance unitaire de 3 à 20 Kw, à une longueur d'onde de 200 à 600 nm, pour durcir la peinture protectrice durcissable aux UV, l'encre durcissable aux UV, et la peinture de fond durcissable aux UV, avec la machine de durcissement UV étant actionnée à une vitesse de transport de 1 à 200 m/min.

14. Utilisation du film de transfert durcissable aux UV selon l'une quelconque des revendications 1 à 6 dans la fabrication d'un panneau décoratif de film de transfert durcissable aux UV.

15. Utilisation selon la revendication 14, comprenant :
l'application d'une couche d'agent de perméation durcissable aux UV sur la surface d'un panneau de ciment renforcé de fibres, un panneau de silicate de calcium renforcé de fibres, un panneau d'oxyde de magnésium renforcé de fibres, un panneau de ciment de chlorure de magnésium léger, un panneau d'oxychlorure de magnésium, ou un panneau de gypse, l'application d'une couche de charge de peinture durcissable aux UV sur la surface de l'agent de perméation durcissable aux UV, l'application d'une couche d'apprêt d'étanchéité durcissable aux UV sur la surface de la charge de peinture durcissable aux UV, l'application d'une couche de peinture pigmentée durcissable aux UV sur la surface de l'apprêt d'étanchéité durcissable aux UV, l'application d'une couche de colle durcissable aux UV sur la surface de la peinture pigmentée durcissable aux UV, et le transfert du film de transfert sur la colle durcissable aux UV, pour obtenir le panneau décoratif de film de transfert durcissable aux UV ; ou
l'application d'une couche d'apprêt d'étanchéité durcissable aux UV sur la surface d'un panneau en bois massif, un panneau MDF, ou un panneau de contreplaqué, l'application d'une couche de colle durcissable aux UV sur la surface de l'apprêt d'étanchéité durcissable aux UV, et le transfert du film de transfert sur la surface de la colle durcissable aux UV, pour obtenir le panneau décoratif de film de transfert durcissable aux UV ; ou
l'application d'une couche d'apprêt métallique durcissable aux UV sur la surface d'une plaque d'aluminium, une tôle d'acier, ou une tôle de fer, l'application d'une couche de colle durcissable aux UV sur la surface de l'apprêt métallique durcissable aux UV, et le transfert du film de transfert sur la surface de la colle durcissable aux UV, pour obtenir la plaque décorative de film de transfert durcissable aux UV.
